# EUROPEAN PATENT SPECIFICATION

(11) **EP 0 283 938 B1**
(45) Date of publication and mention of the grant of the patent: **26.08.1992**
(21) Application number: 88104270.9
(22) Date of filing: 17.03.1988
(51) Int. Cl.: G03C 7/327, G03C 1/30

(54) **Silver halide color photographic material**
Silberhalogenidhaltiges photographisches Farbmaterial
Matériau photographique couleur à l'halogénure d'argent

(30) Priority: 20.03.1987 JP 66708/87; 20.03.1987 JP 66709/87
(43) Date of publication of application: 28.09.1988
(73) Proprietor: Fuji Photo Film Co., Ltd., Kanagawa-ken (JP)
(72) Inventor: Hirano,Tsumoru, Minami Ashigara-shi, Kanagawa-ken (JP); Okamura,Hisashi, Minami Ashigara-shi, Kanagawa-ken (JP); Ono,Shigetoshi, Minami Ashigara-shi, Kanagawa-ken (JP); Sakanoue,Kei, Minami Ashigara-shi, Kanagawa-ken (JP)
(74) Representative: Grünecker, Kinkeldey, Stockmair & Schwanhäusser Anwaltssozietät

(56) References cited:
- EP-A- 0 133 262
- EP-A- 0 161 626
- DE-A- 3 233 168
- DE-A- 3 516 945
- PATENT ABSTRACTS OF JAPAN, vol. 10, no. 195 (P-475)[2251], 9th July 1986; & JP-A-61 39 044 (KONISHIROKU PHOTO IND. CO., LTD.) 25-02-1986
- PATENT ABSTRACTS OF JAPAN, vol. 10, no. 322 (P-511)[2378], 31st October 1986; & JP-A-61 128 241 (FUJI PHOTO FILM CO., LTD.) 16-06-86
- PATENT ABSTRACTS OF JAPAN, vol. 11, no. 267 (C-443)[2714], 28th August 1987; & JP-A-62 68 866 (FUJI PHOTO FILM CO., LTD.) 28-03-87
- PATENT ABSTRACTS OF JAPAN, vol. 11, no. 267 (C-443)[2714], 28th August 1987; & JP-A-62 68 867 (FUJI PHOTO FILM CO., LTD.) 28-03-87

## Description

The present invention relates to color photographic materials that contain a rapid-acting hardener and water-soluble polymer couplers containing carboxyl groups and/or amino groups.

After a silver halide photographic material is exposed to light, when it is color-developed, the oxidized primary amine developing agent reacts with dye-forming couplers to form a color image. Generally, in this technique, color reproduction is effected by a subtractive color process in which complementary color images of yellow, magenta, and cyan are formed to reproduce blue green and red.

As yellow dye image-forming agents, for example, acylacetanilide or benzylmethane-type couplers are used; as magenta dye image-forming agents, for example, pyrazolone, pyrazolotriazole, pyrazolobenzimidazole, cayanoacetophenone or indazolone-type couplers are used; and as cyan dye forming agents, for example, phenol or naphthol-type couplers are used.

In multi-layer color photographic materials, to lessen color mixing, which improves the color reproduction, it is necessary to secure the couplers in their respective separate layers, thereby rendering them fast to diffusion. To render couplers fast to diffusion, many techniques have been used.

One method introduces a long-chained aliphatic group into the molecule of couplers to prevent diffusion. The couplers used in this technique are immiscible with aqueous gelatin solutions. Therefore, it is necessary that the couplers are either dissolved in an alkali and added to an aqueous gelatin solution, or they are dissolved in a high-boiling solvent and emulsified and dispersed into an aqueous gelatin solution.

In such a technique, however, the coupler is liable to crystallize out in the emulsion layer. On the other hand, when a high-boiling solvent is used, since the solvent softens the emulsion layer, it has been required to use a large amount of gelatin, which disadvantageously deteriorates the sharpness of the dye image.

Other techniques for rendering couplers fast to diffusion are to polymerize them.

For example, polymer couplers that are prepared by joining reactive couplers to synthesized polymers (e.g., acrylic acid homopolymers, and p-aminostyrene homopolymers) or natural high-molecular compounds (e.g. gelatin) are described in U.S. Patent Nos. 2,698,797, 2,852,381, 2,852,383, and 2,870,712 and Japanese Patent Publication Nos. 16932/1960 and 3661/1969, and polymer couplers that are prepared by copolymerizing couplers synthesized in the form of ethylenically unsaturated monomers with other polymerizable monomers are disclosed in British Patent Nos. 880,206, 955,197, 967,503, 967,504, 995,363, and 1,104,658. The above hydrophilic polymer couplers, however, are insufficiently fast to diffusion, and they are liable to allow colors to mix. Further, in the worst cases, the couplers disadvantageously flow out during the development processing. To overcome, these problems hydrophilic polymer couplers having phenolic hydroxyl groups or active methylene groups were suggested, as described in U.S. Patent Nos. 4,207,109, 4,215,195, and 4,421,915 and Japanese Patent Application (OPI) No. 27139/1983 and 28744/1983. However, polymers of this type are still inadequately fast to diffusion, and the dye images obtained are low in density.

Other techniques using polymer couplers include dispersing, into an aqueous gelatin solution, lipophilic polymer couplers obtained by emulsion polymerization or solution polymerization of coupler monomers, if necessary, together with other copolymerizable components. Emulsion polymerization is described in U.S. Patent Nos. 3,370,952 and 4,080,211. Solution polymerization is described in U.S. Patent No. 3,451,820.

A considerable improvement in sharpness has been obtained using these lipophilic polymer couplers. Difficulties exist, however, in that the color-forming property is not yet satisfactory and the amount of gelatin used cannot be decreased significantly, and still further improvement in sharpness is desired.

On the other hand, in color photographic materials, in the processing temperature at which a color image is formed is atmospheric temperature (20 to 25 °C ) or higher, and currently the processing temperature is 30°C or higher, in general.

However, in high-temperature rapid processing, a hydrophilic colloid, for example gelatin in which silver halides, color couplers, and other additives are dispersed, becomes softened and swollen. As a result, the emulsion layers are likely to be damaged or to exfoliate from the base. Therefore, the emulsion layers must be hardened when processed at high temperatures. This hardening can be accomplished by introducing the emulsion layers first into a hardening bath during the development processing, or by adding a preliminary hardener such as formaldehyde, dialdehyde, and mucochloric acid into the silver halide emulsions during preparation.

It is important in the hardening of photographic layers that the photographic layers reach their maximum hardness as quickly as possible after drying, so as not to change the permeability to the developing solution.

Recently it has become important to use, instead of hardeners that act over a long period of time, those that act quickly. Through a high speed hardening reaction, it is possible to obviate changes in photographic materials during storage and avoid the continuous lowering of permeability to the developing solutions.

The term "a rapid-acting hardener" in this specification and claims means a compound capable of causing gelatin to crosslink within a short time period, if possible during the coating and drying. A maximum crosslink can be attained within 24 h.

Quite interesting rapid-acting hardeners are carbodiimides, which are disclosed in U.S. Patent Nos. 2,938,892 and 3,098,693, a report by E.Schmidt, F.Hitzler, and E.Lahde in Berichte 71,1933 (1938), and in a report by G.Amiard and R.Heymes in Bul. Soc. Chim. France 1360 (1956); dihydroquinone compounds, described in German Patent Application (OLS) No. 2,322,317; carbamoylpyridinium compounds, described in German Patent Application (OLS) Nos. 2,225,230, 2,317,677, and 2,439,551; and carbamoyloxypyridinium compounds, described in German Patent Application (OLS) No. 2,408,814.

One characteristic common to all of these rapid-acting hardeners is that they activate a carboxyl group in gelatin. This action can be illustrated by the known reaction between carbodiimides and a carboxylic acid. In this reaction an N-acylurea or an acid anhydride is used as an active group. For a protein having carboxyl groups and amino groups, the reaction proceeds further and the activated carboxyl group forms a peptide linkage with the amino group. These compounds are, therefore, known as peptide reagents. (See Chemical Review 67, (1967), pages 107 to 152),

In some cases, however, even if the above rapid-acting hardeners are used, conventional silver halide color photographic materials are not necessarily increased in film strength. Further, silver halide color photographic materials in which all performances such as color-forming property, film strength, and nondiffusibility are satisfactory are not yet available.

DE-A-3516945 discloses a silver halide color photographic material which comprises a hardener that acts by activating a carboxyl group and at least one polymer coupler having a butyl acrylate unit.

It is the object of the invention to provide a silver halide color photographic material that is excellent in fastness of the couplers to diffusion, good in color reproduction, which produces dye images of high density and wherein the film strength is high and the sharpness of an image is remarkably improved by making the film thinner.

This object can be attained by a silver halide color photographic material which comprises a hardener that acts by activating a carboxyl group and at least one polymer coupler comprising at least one repeating unit of the following formula (I): wherein A represents a vinyl polymer unit having a color coupler residue capable of coupling with the oxidized product of an aromatic primary amine developing agent, characterized in that said polymer coupler further has at least one repeating unit of the following formula (II): wherein B represents a vinyl monomer unit having at least one group selected from an amino group and -COOM, wherein M represents a hydrogen atom, an alkali metal or ammonium, and that said polymer coupler is water-soluble.

In the present invention the vinyl monomer unit represented by formula (II) may have both -COOM and an amino group in the unit.

In the present invention, the water-soluble polymer couplers contained in the silver halide photographic material are formed from at least one carboxyl-group-containing monomer or at least one amino-group-containing monomer as a monomer unit. The hardener that activates a carboxyl group in gelatin has the function of reacting with gelatin to form a crosslinkage, so that said polymer couplers may be prevented from diffusing in a constitutional layer or between constitutional layers. Thus the disadvantages hitherto involved can be obviated.

Preferable examples of monomer units represented by formula (I) capable of coupling with the oxidized product of an aromatic primary amine developing agent to form a dye are those represented by formula (III):
wherein R represents a hydrogen atom, a chlorine atom, or an alkyl group having 1 to 4 carbon atoms; D represents -COO-, -CONR'-, or a substituted or unsubstituted phenyl group; E represents a substituted or unsubstituted alkylene group, phenylene group, or aralkylene group; F represents -CONR'-, -NR'CONR'-, -NR'COO-, -NR'CO-, -OCONR'-, -NR'-, -COO-, -OCO-, -CO-, -O-, -S0₂-, -NR'S0₂, or -S0₂NR'-, in which R' represents a hydrogen atom or a substituted or unsubstituted alkyl group or aryl group, and if two or more R' are in the same molecule, they may be the same or different. As substituents in D, E, and R' can be mentioned an alkyl group (e.g., methyl and ethyl), an alkoxy group (e.g., methoxy group and ethoxy group), an aryloxy group (e.g., phenyloxy), an alkoxycarbonyl group (e.g., methoxycarbonyl), an acylamino group (e.g., acetylamino), a carbamoyl group, an alkylcarbamoyl group (e.g., methylcarbamoyl, and ethylcarbamoyl), a dialkylcarbamoyl group (e.g., dimethylcarbamoyl), an arylcarbamoyl group (e.g., phenylcarbamoyl), an alkylsulfonyl group (e.g., methylsulfonyl), an arylsulfonyl group (e.g., phenylsulfonyl), an alkylsulfonamido group (e.g., methanesulfonamido), an arylsulfonamido group (e.g., phenylsulfonamido), a sulfamoyl group, an alkylsulfamoyl group (e.g., ethylsulfamoyl), a dialkylsulfamoyl group (e.g., dimethylsulfamoyl), an alkylthio group (e.g., methylthio), an arylthio group (e.g., phenylthio), a cyano group, a nitro group, and a halogen atom (e.g., fluorine, chlorine, and bromine). If there are two or more substituents they may be the same or different. î, m, and n are 0 or 1, provided that î, m, and n are not 0 at the same time, and Q represents a cyan, magenta, or yellow dye forming coupler residue capable of coupling with the oxidized product of an aromatic primary amine developing agent to form a dye.

Of the color coupler residues represented by Q, as cyan forming coupler residues, preferable compounds are represented by phenol type couplers (IV) or (V), or naphthol type couplers (VI) or (VII) (a hydrogen atom other than one positioned at the coupling position or the I-positioned OH group will split off to join with F of formula (III)).
wherein R¹¹ represents a group capable of replacing a hydrogen on a phenol ring or a naphthol ring such as a halogen atom, a hydroxy group, an amino group, a sulfo group, a cyano group, an aliphatic group, an aromatic group, a heterocyclic group, a carbonamido group, a sulfonamido group, a carbamoyl group, a sulfamoyl group, an acyloxy group, an acyl group, an aliphatic oxy group, an aliphatic sulfonyl group, an aromatic oxy group, an aromatic thio group, an aromatic sulfonyl group, a sulfamoylamino group, a nitro group, and an imido group, with R¹¹ having 0 to 3 carbon atoms,
R¹² represents -CONR¹³R'⁴, -NHCOR¹³, -NHCOOR¹⁵, -NHSO₂R¹⁵, -NHCONR¹³R¹⁴, or -NHSO₂R¹³R¹⁴, in which R¹³ or R¹⁴ represents a hydrogen atom, an aliphatic group having 1 to 30 carbon atoms (e.g., methyl, ethyl, butyl, methoxyethyl, n-decyl, n-dodecyl, n-hexadecyl, trifluoromethyl, heptafluoropropyl, dodecyloxypropyl, 2,4-di-tert-amylphenoxypropyl, and 2,4-di-tert-amylphenoxybutyl), an aromatic group having 6 to 30 carbon atoms (e.g., phenyl, tolyl, 2-tetradecyloxyphenyl, pentafluorophenyl, and 2-chloro-5-dodecyloxycarbonylphenyl), or a heterocyclic group having 2 to 30 carbon atoms (e.g., 2-pyridyl, 4-pyridyl, 2-furyl, and 2-thienyl), R¹⁵ represents an aliphatic group having 1 to 30 carbon atoms (e.g., methyl, ethyl, butyl, dodecyl, and hexadecyl), an aromatic group having 6 to 30 carbon atoms (e.g., phenyl, tosyl, 4-chlorophenyl, and naphthyl), or a heterocyclic group (e.g., 4-pyridyl, quinolyl, and 2-furyl), and R¹³ and R¹⁴ may bond together to form a heterocyclic ring (e.g., morpholine, piperidine, and pyrrolidine), p' is an integer of 0 to 3, q' is an integer of 0 to 2, r' and s' are each integers of 0 to 4,
X represents an oxygen atom, a sulfur atom, or R¹⁶ N , in which R¹⁶ represents a hydrogen atom or a monovalent group such as an aliphatic group having 1 to 30 carbon atoms (e.g., methyl, ethyl, butyl, methoxyethyl, and benzyl), an aromatic group having 6 to 30 carbon atoms (e.g., phenyl, and tolyl), a heterocyclic group having 2 to 30 carbon atoms (e.g., 2-pyridyl, and 2-pyrimidyl), a carbonamido group having 1 to 30 carbon atoms (e.g., formamido, acetamido, N-methylacetamido, and benzamido), a sulfonamido group having 1 to 30 carbon atoms (e.g., methanesulfonamido, toluenesulfonamido, and 4-chlorobenzenesulfonamido), an imido group having 4 to 30 carbon atoms, -OR¹⁷, -SR¹⁷⁻, -COR17, -CONR¹⁷R¹⁸, -COCOR¹⁷, -COCONR¹⁷R¹⁸, -COOR'⁹, -COCOOR'⁹, -S0₂R'⁹, -S0₂0R'⁹, -S02NR17Rl8, and -NR¹⁷R¹⁸, in which R¹⁷ and R¹⁸, which may be the same or different, each represent a hydrogen atom, an aliphatic group having 1 to 30 carbon atoms (e.g., methyl, ethyl, butyl, dodecyl, methoxyethyl, ethyl, trifluoromethyl, and heptafluoropropyl), an aromatic group having 6 to 30 carbon atoms (e.g., phenyl, tolyl, 4-chlorophenyl, pentafluorophenyl, 4-cyanophenyl, and 4-hydroxyphenyl), or a heterocyclic group having 2 to 30 carbon atoms (e.g., 4-pyridyl, 3-pyridyl, and 2-furyl), and R¹⁷ and R¹⁸ may bond together to form a heterocyclic ring (e.g., a morpholino group, and a pyrrolidino group), and as examples of R¹⁹ can be mentioned substituents defined for R¹⁷ and R¹⁸, excluding a hydrogen atom,
Z¹ represents a hydrogen atom, or a group that can split off by the coupling reaction with the oxidized product of an aromatic primary amine developing agent. As examples can be mentioned a halogen atom (e.g., fluorine, chlorine, bromine and iodine), an aliphatic oxy group having 1 to 30 carbon atoms (e.g., methoxy, ethoxy, 2-hydroxyethyoxy, carboxymethyloxy, 3-carboxypropyloxy, 2-methoxyethoxycarbamoyl- methyloxy, 2-methanesulfonylethoxy, 2-carboxymethylthioethoxy, 2-carboxymethylthioethoxy, and triazolyl- methyloxy), an aromatic oxy group having 6 to 30 carbon atoms (e.g., phenoxy, 4-hydroxyphenoxy, 2-acetoamidophenoxy, 2,4-dibenzenesulfonamidophenoxy, and 4-phenylazophenoxy), a heterocyclic oxy group having 2 to 3 carbon atoms (e.g., 4-pyridyloxy and 1-phenyl-5-tetrazolyloxy), an aliphatic thio group having 1 to 30 carbon atoms (e.g., dodecylthio), an aromatic thio group having 6 to 30 carbon atoms (e.g., 4-dodecylphenylthio), a heterocyclic thio group having 2 to 30 carbon atoms (e.g., 4-pyridylthio and 1-phenyltetrazol-5-ylthio), an acyloxy group having 2 to 30 carbon atoms (e.g., acetoxy, benzoyloxy, and lauroyloxy), a carbonamido group having 1 to 30 carbon atoms (e.g., dichloroacetylamido, trifluoroben- zamido), pentafluorobutaneamido, and pentafluorobenzamido), a sulfonamido group having 1 to 30 carbon atoms (e.g., methanesulfonamido, and toluenesulfonamido), an aromatic azo group having 6 to 30 carbon atoms (e.g., phenylazo, 4-chloroephenylazo, 4-methoxyphenylazo, and 4-pivaloylaminophenylazo), an aliphatic oxycarbonyloxy group having 1 to 30 carbon atoms (e.g., ethoxycarbonyloxy, and dodecyloxycar- bonyloxy), an aromtic oxycarbonyloxy group having 6 to 30 carbon atoms (e.g., phenoxycarbonyloxy), a carbamoyloxy group having 1 to 30 carbon atoms (e.g., methylcarbamoyloxy, dodecylcarbamoyloxy, and phenylcarbamoyloxy), and a heterocyclic ring group having 1 to 30 carbon atoms and connected to the active position of the coupler through the nitroben atom (e.g., succinimido, phthalimido, hydantoinyl, pyrazolyl, and 2-benzotriazolyl), and
Y represents a group of atoms required to form a 5-, 6- or 7-membered ring together with the carbon atom to which Y is connected, and more specifically represents -O-, which may be combined, and wherein R" and R each represent a hydrogen atom, an alkyl group, an aryl group, a halogen atom, an alkyl group, an aryl group, a halogen atom, an alkyloxy group, an alkyloxycarbonyl group, an arylcarbonyl group, an alkylcarbamoyl group, an arylcarbamoyl group, or a cyano group.

Examples of substituents preferably used in the invention are given below.

Preferable substituents represented by R¹¹ include a halogen atom (e.g., fluorine, chlorine and bromine), an aliphatic group (e.g., methyl, ethyl, and isopropyl), a carbonamido group (e.g., acetamido, and benzamido), and a sulfonamido group (e.g., methanesulfonamido, and toluenesulfonamido).

Preferable substituents represented by R¹² include -CONR¹³R¹⁴, such as a carbamoyl group, an ethylcarbamoyl group, a morpholinocarbonyl group, a dodecylcarbamoyl group, a hexadecylcarbamoyl group, a decyloxypropyl group, a dodecyloxypropyl group, and a 2,4-di-tert-amylphenoxybutyl group.

Preferable substituents represented by X include R¹⁶ N , in which R¹⁶ more preferably represents -COR17(e.g., formyl, acetyl, trifluoroacetyl, chloroacetyl, benzoyl, pentafluorobenzoyl, and p-chlorobenzoyl), -COOR¹⁹(e.g., methoxycarbonyl, ethoxycarbonyl, butoxycarbonyl, dodecyloxycarbonyl, methoxyethoxycar- bonyl, and phenoxycarbonyl), -S02R'9(e.g., methanesulfonyl, ethanesulfonyl, butanesulfonyl, hexadecanesulfonyl, benzenesulfonyl, toluenesulfonyl, and p-chlorobenzenesulfonyl), -CONR¹⁷R¹⁸ (e.g., N,N-dimethylcarbamoyl, N,N-diethylcarbamoyl, N,N-dibutylcarbamoyl, morpholinocarbonyl, piperidinocarbonyl, 4-cyanophenylcarbamoyl, 3,4-dichlorophenylcarbamoyl, and 4-methanesulfonylphenylcarbamoyl), and -SO₂NR¹⁷R¹⁸(e.g., N,N-dimethylsulfamoyl, N,N-diethylsulfamoyl, and N,N-dipropylsulfamoyl). More preferably groups represented by R¹⁶ are -COR¹⁷, -COOR¹⁹, and -SO₂R¹⁹.

Preferable groups represented by Z¹ are a hydrogen atom, a halogen atom, an aliphatic oxy group, an aromatic oxy group, a heterocyclic thio group, and an aromatic azo group.

The couplers represented by general formulae (IV), (V), (V'), and (VI) may be combined themselves at the substituent R¹¹, R¹²,X or Z¹ via a divalent or higher valent linking group to become a dimer or higher polymer. In that case, of course, the number of carbon atoms defined for the substituents above does not apply.

Magenta color-forming coupler residues are coupler residues represented by formula (VII), (VIII), (IX), (X), (XI), (XII), and (XIII), and they are connected to F of formula (III) at any part of Ar, Z², and R²⁰ to R³².

wherein Ar represents a known substituent at the first position of a 2-pyrazoline-5-on coupler, for example an unsubstituted or substituted alkyl group (e.g., haloalkyl such as fluoroalkyl, cyanoalkyl, and benzylalkyl); an unsubstituted or substituted aryl group [examples of the substituent are an alkyl group (e.g., methyl and ethyl), an alkoxy group (e.g., methoxy and ethoxy), an aryloxy group (e.g., phenyloxy), an alkoxycarbonyl group (e.g., methoxycarbonyl), an acylamino group (e.g., acethylamino), a carbamoyl group, an alkylcarbamoyl group (e.g., methylcarbamoyl and ethylcarbamoyl), a dialkylcarbamoyl group (e.g., dimethylcarbamoyl), an arylcarbamoyl group (e.g., phenylcarbamoyl), an alkylsulfonyl group (e.g., methylsulfonyl), an arylsulfonyl group (e.g., phenylsulfonyl), an alkylsulfonamido group (e.g., methanesulfonamido), an arylsulfonamido group (e.g., phenylsulfonamido), a sulfamoyl group, an alkylsulfamoyl group(e.g., ethylsulfamoyl), a dialkylsulfamoyl group (e.g., dimethylsulfamoyl), an alkylthio group (e.g., methylthio), an arylthio group (e.g., phenylthio), a cyano group, a nitro group, and a halogen atom (e.g., fluorine, chlorine, and bromine). When the substituents are two or more, they may be the same or different, and particularly preferred examples of substituents are a halogen atom, an alkyl group, an alkoxy group, an alkoxycarbonyl group, and cyano group]; or a heterocyclic group (e.g., triazole, thiazole, benzthiazole, furan, pyridine, quinaldine, benzoxazole, pyrimidine, oxazole, and imidazole).

R²⁰ represents an unsubstituted or substituted anilino group, an unsubstituted or substituted acylamino group (e.g., alkylcarbonamido, phenylcarbonamido, alkoxycarbonamido, and phenyloxycarbonamido), or an unsubstituted or substituted ureido group (e.g., alkylureido and phenylureido). Examples of the substituents of these substituted groups are a halogen atom (e.g., fluorine, chlorine, and bromine), a straight-chain or branched-chain alkyl group (e.g., methyl, t-butyl, octyl, and tetradecyl), an alkoxy group (e.g., methoxy, ethoxy, 2-ethylhexyloxy, and tetradecyloxy), an acylamino group (e.g., acetamido, benzamido, butaneamido, octaneamido, tetradecaneamido, α-(2,4-di-tert-amylphenoxy)acetoamido, α-(2,4-di-tert-amylphenoxy)-butylamido, α-(3-pentadecyIphenoxy)hexanearnido, a-(4-hydroxy-3-tert-butylphenoxy)tetradecaneamido, 2-oxo-pyrrolidine-1-yl, 2-oxo-5-tetradecylpyrrolidine-1-yl, and N-methyl-tetradecaneamido), a sulfonamido group (e.g., methanesulfonamido, benzenesulfonamido, ethylsulfonamido, p-toluenesulfonamido, octanesul- fonamido, p-dodecylbenzenesulfonamido, and N-methyl-tetradecanesulfonamido), a sulfamoyl group (e.g., sulfamoyl, N-methylsulfamoyl, N-ethylsulfamoyl, N,N-dimethylsulfamoyl, N,N-dihexylsulfamoyl, N-hex- adecylsulfamoyl, N-[3-(dodecyl)-propyl]sulfamoyl, N-[4-(2,4-di-tert-amylphenoxy)butyl]-sulfamoyl, and N-methyl-N-tetradecylsulfamoyl), a carbamoyl group (e.g., N-methylcarbamoyl, N-butylcarbamoyl, N-oc- tadecylcarbamoyl, N-[4-(2,4-di-tert-amylphenoxy)butyl]-carbamoyl, and N-methyl-N-tetradecylcarbamoyl), a diacyl-amino group (N-succinimido, N-phthalimido, 2,5-dioxo-1-hydantoinyl, and 3-(N-acetyl-N-dodecylamino)succinimido), an alkoxycarbonyl group (e.g., methoxycarbonyl, tetradecyloxycarbonyl, and benzyloxycarbonyl), an alkoxysulfonyl group (e.g., methoxysulfonyl, butoxysulfonyl, octyloxysulfonyl, and tetradecyloxysulfonyl), an aryloxysulfonyl group (e.g., phenoxysulfonyl, p-methylphenoxysulfonyl, and 2,4-di-tert-amylphenoxysulfonyl), an alkanesulfonyl group (e.g., methanesulfonyl, ethanesulfonyl, octanesulfonyl, 2-ethylhexylsulfonyl, and hexadecanesulfonyl), an arylsulfonyl group (e.g., benzenesulfonyl and 4-nonylben- zenesulfonyl), an alkylthio group (e.g., methylthio, ethylthio, hexylthio, benzylthio, tetradecylthio, and 2-(2,4-di-tert-amylphenoxy)ethylthio), an arylthio group (e.g., phenylthio and p-trylthio), an alkyl-oxycarbonylamino group (e.g., methoxycarbonylamino, ethyloxycarbonylamino, benzyloxycarbonyl, and hexadecyloxycar- bonylamino), an alkylureido group (e.g., N-methylureido, N,N-dimethylureido, N-methyl-N-dodecylureido, N-hexadecylureido, and N,N-dioctadecylureido), an acylgroup (e.g., acetyl, benzoyl, octadecanoyl, and p-dodecaneamidobenzoyl), a nitro group, a carboxyl group, a sulfo group, a hydroxyl group, or a trichloromethyl group.

Of the above-mentioned substituents, the number of carbon atoms of a substituent defined as an alkyl group is 1 to 36, and that defined as an aryl group is 6 to 38.

_{R21}, _{R22}, _{R23}, _{R24}, _{R}25, _{R}26, _{R}27, _{R}28, _{R}29, R3°, R³¹, and R³² each represent a hydrogen atom, a hydroxyl group, an unsubstituted or substituted alkyl group (wherein the number of carbon atoms is preferably 1 to 20, e.g., methyl, propyl, t-butyl, trifluoromethyl, and tridecyl), an unsubstituted or substituted aryl group (wherein the number of carbon atoms is preferably 6 to 20, e.g., phenyl, 4-t-butylphenyl 2,4-di-t-amylphenyl, and 4-methylphenyl), an unsubstituted or substituted heterocyclic group (e.g., 2-furyl, 2-thienyl, 2-pirimidinyl, and 2-benzothiazolyl), an alkylamino group (wherein the number of carbon atoms is preferably 1 to 20, e.g., methylamino, diethylamino, and t-butylamino), an acylamino group (wherein the number of carbon atoms is preferably 2 to 20, e.g., acetylamino, propylamino, and benzamino), an anilino group (e.g., phenylanilino and 2-chloroanilino), an alkoxycarbonyl group (wherein the number of carbon atoms is preferably 2 to 20, e.g., methoxycarbonyl, butoxycarbonyl, and 2-ethylhexyloxycarbonyl), an alkylcarbonyl group (wherein the number of carbon atoms is preferably 2 to 20, e.g., acetylcarbonyl, butylcarbonyl, and cyclohexylcarbonyl), an arylcarbonyl group (wherein the number of carbon atoms is preferably 7 to 20, e.g., benzoyl and 4-t-butylbenzoyl), an alkylthio group (wherein the number of carbon atoms is preferably 1 to 20, e.g., methylthio, octylthio, and 2-phenoxyethylthio), an arylthio group (wherein the number of carbon atoms is preferably 6 to 20, e.g., phenylthio and 2-butoxy-5-t-octylphenylthio), a carbamoyl group (wherein the number of carbon atoms is preferably 1 to 20, e.g., N-ethylcarbamoyl, N,N-dibutylcarbamoyl, and N-methyl-N-butylcarbamoyl), a sulfamoyl group (wherein the number of carbon atoms is preferably 20 or below, e.g., N-ethylsulfamoyl, N,N-di-ethylsulfamoyl, and N,N-dipropylsulfamoyl), or a sulfonamido group (wherein the number of carbon atoms is preferably 1 to 20, e.g., methanesulfonamido, benzenesulfonamido, and p-toluenesulfonamido).

Z² represents a hydrogen atom or a group which can split-off upon a coupling-reaction with the oxidation product of an aromatic primary amine developing agent. Examples of such split-off groups include a halogen atom (e.g., chlorine atom and bromine atom), a split-off group connected through the oxygen atom (e.g., acetoxy, propanoyloxy, benzoyloxy, ethoxyoxazoyloxy, pyruvinyloxy, cinnamoyloxy, pheoxy, 4-cyanophenoxyl, 4-titaniumsulfonamidophenoxy, a-naphtoxy, 4-cyanoxyl, 4-methanesulfonamido-phenoxy, 3-pentadecylphenoxy, benzyloxycarbonyloxy, ethoxy, 2-cyanoethoxy, benzyloxy, 2-phenethyloxy, 2-phenoxy- ethoxy, 5-phenyltetrazoyloxy, and 2-benzothiazolyloxy), a split-off group connected through the nitrogen atom (e.g., the groups described in Japanese Patent Application (OPI) No. 189538/1982 or benzenesulfonamido, N-ethyltoluenesulfonamido, heptafluorobutaneamido, 2,3,4,5,6-pentafluorobenzamido, octanesul- fonamido, p-cyanophenylureido, N,N-diethylsulfamoylamino, 1-piperidyl, 5,5-dimethyl-2,4-dioxo-3-ox- azolydinyl, 1-benzyl-5-ethoxy-3-hydantoinyl, 2-oxo-1,2-dihydro-l-pyrizonyl, imidazolyl, pyrazolyl, 3,5-diethyl-1,2,4-triazole-1-yl, 5-or 6-bromobenzotriazole-1-yl, 5-methyl-1,2,3,4-triazole-1-yl, and benzimidazolyl), and a split-off group connected through the sulfur atom (e.g., phenylthio, 2-carboxyphenylthio, 2-methoxy-5-octylphenylthio, 4-methanesulfonylphenylthio, 4-octanesulfonamidophenylthio, benzylthio, 2-cyanoethylthio, 5-phenyl-2,3,4,5-tetrazoylthio, and 2-benzothiazolyl). Preferred examples of split-off groups include a halogen atom, a phenoxy group, and a split-off group connected through the nitrogen atom. Particularly preferred examples include a halogen atom, phenoxy group, pyrazolyl group, imidazolyl group, and triazolyl group.

As a residue of yellow color-forming couplers, an acylacetoanilido type is preferable, and a pivaloylacetoanilido type (XIV), or a benzoylacetoanilido type (XV) or (XVI) is even more preferable.

wherein R³³, R³⁴, R³⁵, and R³⁶, which may be the same or different, each represent a hydrogen atom or a known substituent of the residue of a yellow color-forming coupler (e.g., alkyl, alkenyl, alkoxy, alkoxycarbonyl, halogen atom, alkoxycarbamoyl, aliphatic amino, alkylsulfamoyl, alkylsulfonamido, alkylureido, alkyl-substituted succinimido, aryloxy, aryloxycarbonyl, arylcarbamoyl, arylamido, arylsulfamoyl, arylsulfonamido, arylureido, carboxyl, sulfo, nitro, cyano, and thiocyano).

Z³ represents a hydrogen atom or a group represented by the following formulas (XVII), (XVIII), (XIX), or (XX).

wherein R³⁷ represents an aryl group or a heterocyclic group which may be substituted.

wherein R³⁸ and R³⁹, which may be the same or different, each represent a hydrogen atom, a halogen atom, an ester group of carboxylate, an amino group, an alkyl group, an alkylthio group, an alkoxy group, an alkylsulfonyl group, an alkylsulfinyl group, a carboxylic group, a sulfon group, an unsubstituted or substituted phenyl or heterocyclic group.

wherein W¹ represents a non-metal atom necessary to form a 4- or 5-membered ring with in the formula.

Preferred examples of compounds represented by formula (XX) include those represented by the following formulas (XXI) - (XXIII):

wherein R⁴° and R41 each represent a hydrogen atom, an alkyl group, an aryl group, an alkoxy group, an aryloxy group, or a hydroxyl group; R⁴², R⁴³, and R⁴⁴ each represent a hydrogen atom, an alkyl group, an aryl group, an alalkyl group, or an acyl group; and W₂ represents an oxygen atom or a sulfur atom.

Preferred examples of the monomer unit containing a carboxyl group or an amino group represented by formula (II) include compounds represented by the following formula (XXIVa) or (XXIVb):

wherein R⁴⁵ represents a hydrogen atom, a lower alkyl group having 1 to 4 carbon atoms, or a chlorine atom; P represents -COO-, -CONHR⁴⁶'-, or a substituted or unsubstituted phenylene group; T represents -COO-, -CONH-, or a substituted or unsubstituted phenylene group; L represents a substituted or unsubstituted alkylene, a phenylene or an aralkylene group; M represents a hydrogen atom, an alkali metal or ammonium; m' and n' each represent 0 or 1; R⁴⁶ and R⁴⁶' each represent a hydrogen atom, or a substituted or unsubstituted alkyl or aryl group. The substituents contained in P, T, L, R⁴⁶ and R⁴⁶', which may be the same or different, if there are two or more present, include an alkyl group (e.g., methyl and ethyl), an alkoxy group (e.g., methoxy and ethoxy), an aryloxy group (e.g., phenyloxy), an alkoxycarbonyl group (e.g., methoxycarbonyl), an acylamino group (e.g., acetylamino), a carbamoyl group, an alkylcarbamoyl group (e.g.,methylcarbamoyl and ethylcarbamoyl), a dialkyl-carbamoyl group (e.g., dimethylcarbamoyl), an arylcarbamoyl group (e.g., phenylcarbamoyl), an alkylsulfonyl group (e.g., methylsulfonyl), an arylsulfonyl group (e.g., phenylsulfonyl), an alkylsulfonamido group (e.g., methanesulfonamido), an arylsulfonamido group (e.g., phenylsulfonamido), a sulfamoyl group, an alkylsulfamoyl group (e.g., ethylsulfamoyl), a dialkylsulfamoyl group (e.g., dimethylsulfamoyl), an alkylthio group (e.g., methylthio), an arylthio group (e.g., phenylthio), a cyano group, a nitro group, and a halogen atom (e.g., fluorine, chlorine, and bromine).

Specific examples of monomer units representing formula (XXIVa) are given below.

The above-mentioned water-soluble polymer coupler to be used in the present invention may contain a non-color-forming ethylenically-unsaturated monomer unit which does not undergo a coupling reaction with the oxidation product of an aromatic primary amine developing agent other than those represented by formulas (I) and (II), and which does not contain -COOM or an amino group in the molecule. The amount of such monomer unit is in the range between 0 to 60%, in a weight ratio to the polymer coupler represented by formula (I) or (II).

As a non-color-forming ethylenically-unsaturated monomer unit which does not undergo a coupling reaction with the oxidation product of an aromatic primary amine developing agent other than those represented by formulas (I) and (II), the following examples may be mentioned; acrylate esters, methacrylate esters, crotonate esters, vinyl esters, maleate diester, fumarate diesters, itaconate diesters, acrylamides, methacrylamides, vinyl ethers, and styrenes.

Examples of such monomers include acrylate esters such as methyl acrylate, ethyl acrylate, n-propyl acrylate, isopropyl acrylate, n-butyl acrylate, isobutyl acrylate, tert-butyl acrylate, hexyl acrylate, 3-acroyl- propanesulfonic acid, acetoacetoxyethyl acrylate, acetoxyethyl acrylate, phenyl acrylate, 2-methoxy acrylate, 2-ethoxy acrylate, and 2-(2-methoxyethoxy)ethyl acrylate; methacrylate esters such as methyl methacrylate, ethyl methacrylate, n-propyl methacrylate, n-butyl methacrylate, tert-butyl methacrylate, cyclohexyl methacrylate, 2-hydroxyethyl methacrylate, and ethoxyethyl methacrylate; crotonate esters such as butyl crotonate and hexyl crotonate; vinyl esters such as vinyl acetate, vinyl propionate, vinyl butylate, vinylmethoxy acetate, and vinyl benzoate; maleate diesters such as diethyl maleate, dimethyl maleate, and dibutyl maleate; fumarate diesters such as diethyl fumarate, dimethyl fumarate, and dibutyl fumarate; itaconate diesters such as diethyl itaconate, dimethyl itaconate, and dibutyl itaconate; acrylamides such as acrylamide, methyl acrylamide, ethyl acrylamide, isopropyl acrylamide, n-butyl acrylamide, hydroxylmethyl acrylamide, diacetone acrylamide, acryloyl morpholine, and acrylamido-2-methylpropanesulfonate; methacrylamides such as methyl methacrylamide, ethyl methacrylamide, n-butyl methacryamide, tert-butyl mathacrylamide, 2-methoxy methacrylamide, dimethyl methacryamide, and diethyl methacrylamide; vinyl ethers such as methyl vinyl ether, butyl vinyl ether, hexyl vinyl ether, methoxyethyl vinyl ether, and dimethylaminoethyl vinyl ether; and styrenes such as styrene, methyl styrene, dimethyl styrene, trimethyl styrene, triethyl styrene, isopropyl styrene, butyl styrene, chloromethyl styrene, methoxy styrene, butoxy styrene, acetoxy styrene, chlorostyrene, dichlorostyrene, bromostyrene, 2-methyl styrene, vinyl benzoic- methyl ester, styrenesulfonic acid, and styrenesulfinic acid.

Examples of other monomers include allyl compounds (e.g., ally] acetates), vinyl ketones (e.g., methyl vinyl ketone), vinyl heterocyclic compounds (e.g., vinylpyridine), glycidyl esters (e.g., glycidyl acrylate), unsaturated nitriles (e.g., acrylonitrile), monoalkyl itaconate (e.g., monometyl itaconate), monoalkyl maleate (monomethyl maleate), vinylsulfonic acid, acryloyloxyalkylsulfonate (e.g., acryloyloxypropanesulfonate), and acrylamidoalkylsulfonate (e.g., 2-acrylamido-2-methylpropanesulfonate). These acids may be the salts of an alkali metal (e.g., Na, and K) or an ammonium ion.

Of these monomers, preferred comonomers in view of hydrophilic, lipophilic or copolymerization properties of the monomer, the color developing property of the coupler formed, the oil pKa', and the tone of dye formed, include acroyloxyalkylsulfonate, methacryloy-loxyalkylsulfonate, acrylamidoalkylsulfonate, methacryl-amidoalkylsulfonate, and the alkali metal or ammonium salts of these acids.

Monomers that are highly hydrophilic are particularly preferable. Two or more of these monomers may be combined. Examples of combinations thereof include potassium styrenesulfinate/sodium acrylamide-2-methylpropanesulfonate, acetoacetoxyethyl methacrylate/sodium 3-acryloylpropanesulfonate, potassium styrenesulfinate/butyl acrylate/sodium styrenesulfonate, and potassium styrensulfonate/sodium acryloyloxypropanesulfonate.

Although it is desired that the proportion of the color-forming moiety corresponding to formula (I) in the polymer couplers used in the present invention (in terms of the total of those corresponding to formula (I) and (II) and, ethylenically-unsaturated comonomer unit other than those of formula (I) and (II) if contained) is usually 5 to 80 wt. %, in view of the color reproduction, the color formation, and the stability, this proportion is preferably 20 to 70 wt. %. It is preferable that the proportion of the part (monomer unit) corresponding to formula (II) in the polymer couplers used in the present invention is 95 to 20 wt.%, more preferably 2 to 30 wt.%. In this case, the molecular weight equivalent (the gram of a polymer containing 1 mol of a monomer coupler) is about 250 to 4000, but it is not limited to that.

The polymer coupler used in the present invention is added in an amount of 0.005 to 0.5 mol, preferably 0.01 to 0.1 mol per mol of silver, to a silver halide emulsion layer in terms of the coupler monomer unit represented by formula (I).

It is preferable that the molecular weight of the polymer coupler used in the present invention is 5 x 10³ to 1 x 10⁷. If the molecular weight is too low, the polymer moves easily, whereas if the molecular weight is too high, difficulty will sometimes arise in the coating process. More preferably the molecular weight is 1 x 10⁴ to 2 x 10⁶.

The synthesis of the water-soluble couplers used in the present invention may be effected by using, as a polymerization initiator and a polymerization solvent, compounds described in Japanese Patent Application (OPI) Nos. 120252/1983, 145944/1983, 211756/1983, 224352/1983, 42543/1984, 171956/1984, 228252/1984, 35732/1985 and 46555/1985.

The water-soluble polymer couplers used in this invention can be synthesized by a solution polymerization method. As the solvent for polymerization, a solvent having a low coefficient value of chain transfer to a radical not reacting with a polymerization initiator is preferred. Examples of such a solvent, which may be used by mixing two or more, include water, toluene, alcohols (e.g., methanol, ethanol, isopropyl alcohol, and t-butanol), tetrahydrofuran, dioxane, ethyl acetate, dimethylformamide, dimethylacetoamide, and dimethylsulfoxide.

It is necessary to set the polymerization temperature in association with the molecular weight of the polymer that will be produced, the type of the initiator, and so on, and although polymerization may be carried out in the range of between 0 ° C and 100 C, it is generally carried out in the range of 30 to 100 ° C.

As the water-soluble polymerization initiator, for example, salts of persulfuric acid such as potassium persulfate, ammonium persulfate, sodium persulfate; water soluble azo compounds such as sodium 4,4'-azobis-4-cyanovalerate, and 2,2'-azobis(2-amidinopropane) hydrochloride; and hydrogen peroxide can be used. As the lipophilic polymerization initiator, it can be mentioned, for example, lipophilic azo compounds such as azobisisobutyronitrile, 2,2'-azobis-(2,4-dimethylvaleronitrile), 2,2'-azobis(4-methoxy-2,4-dimethylvaleronitrile), dimethyl 2,2'-azobisisobutyrate, and 4,4'-azobis-4-cyanovalerate; and lipophilic peroxides such as benzoyl peroxide, lauryl peroxide, chlorobenzyl peroxide, diisopropyl peroxydicarbonate, and di-t-butyl peroxide. Of these, benzoyl peroxide, chlorobenzyl peroxide, and lauryl peroxide are preferable.

These polymerization intiators can be used in an amount of 0.01 to 10 wt.%, preferably 0.1 to 5 wt.%, based on the total amount of monomers.

The term "water-soluble" in this specification and claims means that the obtained polymer coupler will dissolve into water in an amount of 1.0 wt. % or more. In view of the production it is preferable that the obtained polymer coupler dissolves into water in an amount of 10 wt. % or more.

It is possible that the polymer coupler can be added as an aqueous solution to a coating fluid, or that it can be dissolved in a solvent mixture of water and an organic solvent miscible with water, such as lower alcohols, THF, acetone, and ethyl acetate, and then added to a coating fluid.

Further, the polymer coupler can be dissolved in an aqueous alkali solution or an aqueous-alkali- containing organic solvent mixture and then added to a coating fluid. It is also possible to add a small quantity of a surface-active agent.

In any case, it is considered that the water-soluble polymer coupler used in the present invention does not take the form of oil droplets or a latex in the coating fluid or in the coating film, but interacts with the hydrophilic binder, thereby each solubilizing the other to some degree.

Therefore, it is considered that the film strength exhibits excellent performance in comparison with oil-soluble (with latex type inclusive) polymer couplers.

Examples of the water-soluble polymer couplers used in the present invention are shown below.

As preferable examples of carboxyl-group-activating-type hardeners used in the present invention can be mentioned compounds represented by the following formulae (XXV) to (XXXIII):
wherein R⁴⁷ and R⁴⁸, which may be the same or different, each represent an alkyl group having 1 to 10 carbon atoms (e.g., methyl, ethyl, and 2-ethylhexyl), an aryl group having 6 to 15 carbon atoms (e.g., phenyl and naphthyl), or an aralkyl having 7 to 15 carbon atoms (e.g., benzyl and phenetyl). It is preferable that R⁴⁷ and R⁴⁸ bond together with the nitrogen atom to form a heterocyclic ring, such as a pyrrolidine ring, a piperazine ring, and a morpholine ring. R⁴⁹ represents a substituent such as a hydrogen atom, a halogen atom, a carbamoyl group, a sulfo group, a ureido group, an alkoxy group and an alkyl group having 1 to 10 carbon atoms. If R⁴⁹ represents an alkoxy group or an alkyl group, then the group may further have a substituent such as a halogen atom, a carbamoyl group, a sulfo group, and a ureido group. X⁸ represents an anion and becomes a counter ion to the N-carbamoylpyridinium salt. If the substituent of R⁴⁹ contains a sulfo group, an inner salt is formed and X⁸ may not be present. Preferable examples of the anions include halide ions, a sulfonic ion, a sulfonate ion, CℓO₄^{e}, BF₄⁸ and PF₆^{e.}
wherein _{R}⁴⁷, _{R}⁴⁸, R⁴⁹ and X^{e} have the same meaning as defined in formula (XXVII).
wherein R⁵⁰, R⁵¹, R⁵², and R⁵³, which may be the same or different, each represent an alkyl group having 1 to 20 carbon atoms (e.g., methyl, ethyl, butyl, 2-ethylhexyl, and dodecyl), an aralkyl having 6 to 20 carbon atoms (e.g., benzyl, phenetyl, and 3-pyridylmethyl) or an aryl group having 5 to 20 carbon atoms (e.g., phenyl, naphthyl, and pyridyl), and each may have a substituent such as a halogen atom, an alkoxy group having 1 to 20 carbon atoms, an aryloxy group having 6 to 20 carbon atoms, and an N,N-disubstituted carbamoyl group.
It is also preferable that any two of R⁵⁰, R⁵¹, R⁵², and R⁵³ bond together to form a ring. Examples of rings formed by bonding R⁵⁰ and R⁵¹ or R⁵² and R⁵³ together with the nitrogen atom include a pyrrolidine ring, a piperazine ring, a perhydroazepine, and a morpholine ring. Examples of rings formed by bonding R⁵⁰ and R⁵² or R⁵¹ and R⁵³ together with the two nitrogen atoms and the carbon atom between them include an imidazoline ring, a tetrahydropyrimidine ring, and a tetrahydrodiazepine ring.
X represents a group that can split off when the compound represented by formula (XXVII) reacts with a nucleophilic reagent, preferable examples being a halogen atom, a sulfonyloxy group, and a 1-pyridiniumyl group.
Y^{e} represents an anion, preferably a halide ion, a sulfonate ion, a sulfuric acid ion, Cℓ₄^{e}, BF₄⁸ or PF₆^{e} , and if Y^{e} represents a sulfonate ion, it may bond to X, R⁵⁰, R⁵¹, R⁵² or R⁵³ to form an inner salt.
wherein R⁵⁴ represents an alkyl group having 1 to 10 carbon atoms (e.g., methyl, ethyl, and 2-ethylhexyl), a cycloalkyl group having 5 to 8 carbon atoms (e.g., cyclohexyl), an alkoxyalkyl group having 3 to 10 carbon atoms (e.g., methoxyethyl), an aralkyl group having 7 to 15 carbon atoms (e.g., benzyl and phenetyl); R⁵⁴' represents the groups defined for R⁵⁴, or preferably R⁵⁵ represents an alkylene group having 2 to 4 carbon atoms (e.g., ethylene, propylene, and trimethylene); R⁵⁶ and R⁵⁷, which may be the same or different, each represent an alkyl group having 1 to 6 carbon atoms (e.g., methyl and ethyl). It is also preferable that R⁵⁶ and R⁵⁷ bond together with the nitrogen atom to form a heterocyclic ring (e.g., pyrrolidine, piperazine, and morpholine). R⁵⁸ represents an alkyl group having 1 to 6 carbon atoms (e.g., methyl, ethyl, and butyl), wherein it is also preferable if it is substituted by a substituted or unsubstituted carbamoyl group or a sulfo group; X^{a} represents an anion, preferably a halide ion, a sulfonate ion, a sulfuric acid ion, CℓO₄^{e}, BF₄^{e} or PF₆^{e} ; and if R⁵⁸ is substituted by a sulfo group, an inner salt is formed and X^{a} may not be present.
R⁵⁹ represents an alkyl group having 1 to 10 carbon atoms (e.g., methyl, ethyl, and butyl), an aryl group having 6 to 15 carbon atoms (e.g., phenyl and naphthyl), or an aralkyl group having 7 to 15 carbon atoms (e.g., benzyl and phenetyl), which may be substituted, for example, by a carbamoyl group, a sulfamoyl group, or a sulfo group; R⁶⁰ and R⁶¹, which may be the same or different, each represent a substituent such as a hydrogen atom, a halogen atom, an acylamido group, a nitro group, a carbamoyl group, a ureido group, an alkoxy group, an alkyl group, an alkenyl group, an aryl group, and an aralkyl group. It is also preferable that R⁶⁰ and R⁶¹ bond together with the pyridinium ring skeleton to form a condensed ring.
X represents a group that can split off when the compounds represented by formula (XXIX) react with a nucleophilic reagent, preferable examples being a halogen atom, a sulfonyloxy group, or a group represented by in which R⁶² represents an alkyl group or an aryl group. If X represents a sulfonyloxy group, it is preferable that X and R⁵⁹ bond together.
Y represents an anion, preferably a halide ion, a sulfonate ion, a sulfuric acid ion, CℓO₄^{e} BF₄^{e} or PF₆^{e} , and if R⁵⁹ is substituted by a sulfo group, an inner salt is formed and Y^{e} may not be present.
wherein ^{R63} and ^{R64} have the same meaning as defined for ^{R47} and ^{R48} of formula (XXV), _{R}65 represents an alkyl group having 1 to 10 carbon atoms (e.g., methyl, ethyl, and butyl), an aryl group having 6 to 15 carbon atoms (e.g., phenyl and naphthyl), or an aralkyl group having 7 to 15 carbon atoms, and X⁸ represents an anion, preferably a halide ion, a sulfonate ion, a sulfuric acid ion, C104.", BF₄⁸, or PF₆⁸.
wherein R⁶⁶ preferably represents a straight-chain or branched alkyl group having 1 to 20 carbon atoms (e.g., methyl, ethyl, butyl, 2-ethylhexyl, and dodecyl), an aralkyl group having 7 to 20 carbon atoms (e.g., benzyl and phenetyl), an aryl group having 6 to 20 carbon atoms (e.g., phenyl and naphthyl), an alkenyl group having 2 to 20 carbon atoms (e.g., vinyl and propenyl), or a heteroaromatic ring group (e.g., pyridyl and quinolyl), and it may have a substituent such as a halogen atom, a nitro group, an alkoxy group having 1 to 20 carbon atoms, and an aryloxy group having 2 to 20 carbon atoms. If R⁶⁶ represents a heteroaromatic ring group, it bonds via its carbon atom to in which R⁶⁷ and R⁶⁸ preferably represent a straight-chain or branched alkyl group having 1 to 20 carbon atoms (e.g., methyl, ethyl, butyl, 2-ethylhexyl, or dodecyl), an aralkyl group having 7 to 20 carbon atoms (e.g., benzyl and phenetyl), an aryl group having 6 to 20 carbon atoms (e.g., phenyl group and naphthyl), an alkenyl group having 2 to 20 carbon atoms (e.g., vinyl and propenyl), or a heteroaromatic ring group (e.g., pyridyl and quinolyl), and each may have a substituent such as a halogen atom, a nitro group, an alkoxy group having 1 to 20 carbon atoms, an aryloxy group having 6 to 20 carbon atoms, an alkyl group having 1 to 20 carbon atoms, and an aryl group having 6 to 20 carbon atoms, and they may bond together with the nitrogen atom to form a heterocyclic ring, preferable examples being a pyrrolidine ring, a piperidine ring, and a morpholine ring.
X represents a group that can split off when the compounds represented by formula (XXXI) react with a nucleophilic reagent, examples being a halogen atom (e.g., chlorine and bromine), a phthalimidyloxy group, a succinimidyloxy group, a glutarimidyloxy group, an azoryloxy group (e.g., 1-benzotriazolyloxy), an ammonio group (e.g., 1-pyridinio and 1-quinolinio), an alkylsulfonyloxy group having 1 to 20 carbon atoms, and an arylsulfonyloxy group having 6 to 20 carbon atoms, and X may be substituted by a substituent, preferably, for example, by a halogen atom, a nitro group, a sulfo group, a carbamoyl group, an alkyl group having 1 to 20 carbon atoms, an aryl group having 6 to 20 carbon atoms, an alkoxy group having 1 to 20 carbon atoms, or an aryloxy group having 6 to 20 carbon atoms.
wherein R⁶⁹ and R⁷⁰ preferably represent a straight-chain or branched alkyl group having 1 to 20 carbon atoms (e.g., methyl, ethyl, butyl, 2-ethylhexyl, and dodecyl), a cycloalkyl group having 3 to 20 carbon atoms (e.g., cyclopropyl and cyclohexyl), an aralkyl group having 7 to 20 carbon atoms (e.g., benzyl and phenetyl), an aryl group having 6 to 20 carbon atoms (e.g., phenyl and naphthyl), an alkenyl group having 2 to 20 carbon atoms (e.g., vinyl and propenyl), or a heterocyclic group (e.g., pyridyl), and they may have a substituent such as a halogen atom, a nitro group, an alkoxy group having 1 to 20 carbon atoms, and an aryloxy group having 6 to 20 carbon atoms. The ring formed by bonding R⁶⁹ and R⁷⁰ together preferably should be a pyrrolidine ring, a piperidine ring, or a morpholine ring,
R⁷¹ preferably represents a straight-chain or branched alkyl group having 1 to 20 carbon atoms (e.g., methyl, ethyl, butyl, 2-ethylhexyl, and dodecyl), a cycloalkyl group having 3 to 20 carbon atoms (e.g., cyclopropyl and cyclohexyl), an aralkyl group having 7 to 20 carbon atoms (e.g., benzyl and phenetyl), an aryl group having 6 to 20 carbon atoms (e.g., phenyl and naphthyl), an alkenyl group having 2 to 20 carbon atoms (e.g., vinyl and propenyl), a heterocyclic group (e.g., pyridyl and quinolyl), or a group and it may have a substituent such as a halogen atom, a nitro group, an alkoxy group having 1 to 20 carbon atoms, and an aryloxy group having 6 to 20 carbon atoms,
R⁷² and R⁷³ preferably represent a straight-chain or branched alkyl group having 1 to 20 carbon atoms (e.g., methyl, ethyl, butyl, 2-ethylhexyl, and dodecyl), an aralkyl group having 7 to 20 carbon atoms (e.g., benzyl and phenetyl), an aryl group having 6 to 20 carbon atoms (e.g., phenyl and naphthyl), or an alkenyl having 2 to 20 carbon atoms (e.g., vinyl and propenyl),
R⁶⁹ and R⁷⁰ or R⁷² and R⁷³ may bond together with the nitrogen atom to form a ring, such as a pyrrolidine ring, a piperidine ring, or a morpholine ring,
X represents a group that can split off when the compounds represented by formula (XXXII) react with a nucleophilic reagent, examples being a halogen atom (e.g., chlorine and bromine), a phthalimidyloxy group, a succinimidyloxy group, a glutarimidyloxy group, an azolyloxy group (e.g., 1-benzotriazolyloxy), an ammonio group (e.g., 1-pyridinio), an alkylsulfonyloxy group having 1 to 20 carbon atoms, and an arylsulfonyloxy group having 6 to 20 carbon atoms, and X may be substituted.

The compound represented by formula (XXXII) may form a salt with an acid, for example, preferably with HCℓ, HBr, HBF₄, HPF₆, HCℓO₄, H₂S0₄, an alkylsulfonic acid having 1 to 20 carbon atoms, or an aryl (heteroaromatic ring) sulfonic acid having 5 to 20 carbon atoms.

wherein _{R}⁷⁴, _{R}⁷⁵, R⁷⁶, R⁷⁷, R⁷⁸, and R⁷⁹, which may be the same or different, each preferably represent a straight-chain or branched alkyl group having 1 to 20 carbon atoms (e.g., methyl, ethyl, butyl, 2-ethylhexyl, and dodecyl), an aralkyl group having 6 to 20 carbon atoms (e.g., benzyl, phenetyl, and 3-pyridylmethyl), or an aryl group having 5 to 20 carbon atoms (e.g., phenyl, naphthyl, and pyridyl), and they may have a substituent such as a halogen atom, an alkoxy group having 1 to 20 carbon atoms, an aryloxy group having 6 to 20 carbon atoms, and an N,N-disubstituted carbamoyl group.

It is also preferable that any two of R⁷⁴, R⁷⁵, R⁷⁶, R⁷⁷, R⁷⁸, and R⁷⁹ bond together to form a ring. For example, _{R}⁷⁴ and _{R}⁷⁵, R⁷⁶ and R⁷⁷, or R⁷⁸ and R⁷⁹ bond together with the nitrogen atom to form a pyrrolidine ring, a piperazine ring, a perhydroazepine ring, a morpholine ring, or a pyrrole ring.

X represents a group that can split off when the compounds represented by formula (XXXIII) react with a nucleophilic reagent, preferable examples being a halogen atom, a sulfonyloxy group, a 1-pyridiniumyl group, an imidyloxy group (e.g., succinimidyloxy, glutarimidyloxy, and phthalimidyloxy), an azoryloxy group (e.g., 1-benzotriazolyloxy).

Y^{e} represents an anion such as a halide ion, a sulfonate ion, a sulfuric acid ion, a phosphonate ion, a phosphoric acid ion, BF₄⁸, CℓO₄^{e} , and PF₆^{e} , with Cℓ^{e}, BF₄⁸ , CRO₄^{e}, PFₛ^{e} , and a sulfonate ion being more preferable.

In addition to the compounds represented by formulae (XXV) to (XXXIII), as carboxyl-group-activating-type hardeners used in the invention, preferable compounds are described in Japanese Patent Application (OPI) Nos. 38540/1975, 93470/1977, 43353/1981, and 113929/1983, and U.S. Patent No. 3,321,313.

Examples of compounds to be used in the present invention are shown below.
a. Exemplified compounds represented by formula (XXV) (The methods for synthesis of these compounds are described in detail in U.S. Patent Nos. 3,880,665 and 4,063,952)
b. Exemplified compounds represented by formula (XXVI) (The methods for synthesis of these compounds are described in detail in U.S. Patent No. 4,055,427.)
c. Exemplified compounds represented by formula (XXVII) (The methods for synthesis of these compounds are described in detail in U.S. Patent No. 4,673,632.)
d. Exemplified compounds represented by formula (XXVIII) (The methods for synthesis of these compounds are described in detail in German Patent Nos. 2,439,553 and 2,545,477.)
e. Exemplified compounds represented by formula (XXIX) (The methods for synthesis of these compounds are described in detail in British Patent No. 1,462,789, Japanese Patent Application (OPI) No. 46538/1982, and Japanese Patent Publication No. 50669/1983.)
f. Exemplified compounds represented by formula (XXX) (The methods for synthesis of these compounds are described in detail in U.S. Patent No. 4,067,741.)
g. Exemplified compounds represented by formula (XXXI) (The methods for synthesis of these compounds are described in detail in Japanese Patent Application (OPI) No. 68866/1987.)
h. Exemplified compounds represented by formula (XXXII) (The methods for synthesis of these compounds are described in detail in Japanese Patent Application (OPI) No. 68867/1987.)
i. Exemplified compounds represented by formula (XXXIII) (The methods for synthesis of these compounds are described in detail in U.S. Patent No. 4,668,616.)
j. Compounds described in U.S. Patent No. 4,013,468.
k. Compounds described in U.S. Patent No. 4,111,926.
ℓ. Compounds described in U.S. Patent No. 4,427,768.
m. Compounds described in Japanese Patent Application (OPI) No. 113929/1983.
n. Compounds described in U.S. Patent No. 3,321,313.

When the hardeners represented by formulae (XXV) to (XXXIII), which act by activating a carboxyl group in gelatin, are used in photographic layers, unfavorable phenomenons such as reactions with couplers contained in color photographic materials, the occurrence of stain, photographic deterioration such as fogging, and desensitization are hardly observed. Further, the progress of the hardening is quick, the final hardness is attained within a few days, and a further increase of the hardness thereafter, that is, posthardening, is not substantially observed.

These compounds have excellent affinity for water and do not require organic solvents when added. Therefore problems such as uneven coating due to the organic solvent do not arise. Also, there is no concern regarding a possible explosion or the like. These compounds have no particular physiological action, and since they are of low vapor pressure, unfavorable effects on the human body are reduced.

The amount of hardener used in the invention can be selected depending on the purpose. Generally the amount can be in the range of 0.01 to 20 wt. %, more preferably in the range of 0.05 to 10 wt. % for dried gelatin.

The hardeners of the present invention can be used for a method of extending the chain length of gelatin by partial hardening, as described in Japanese Patent Application (OPI) No. 2324/1981. The hardeners used in the invention can also be used for hardening gelatin whose chain has thus been lengthened.

The hardeners used in the present invention can be used in any photographic materials that use gelatin, for example, a color negative film, a color reversal film, a color positive film, a color photographic paper, a color reversal photographic paper, a color photographic material used in the color diffusion transfer reversal process or in the silver dye bleaching process, and black and white photographic materials such as a black and white film, an X-ray film, a process film, a black and white photographic paper, an aerial film, a microfilm, a facsimile film, a photocomposing film, a photocomposing photographic paper, and a film for graphs.

There is no particular limit on photographic layers in which the hardener is used, and the hardener can be used not only in a silver halide emulsion layer, but also in any gelatin-containing photographic layer, including such non photosensitive layers as an undercoat layer, a back layer, a filter layer, an intermediate layer, and an overcoat layer.

The hardeners can be used alone or in combination, and they can also be combined with other hardeners known in the art, such as aldehyde-type compounds, for example formaldehyde and glutaraldehyde; ketone compounds, such as diacetyl, cyclopentanedione, bis(2-chloroethylurea), 2-hydroxy-4,6-dichloro-1,3,5-triazine, divinyl sulfon, 5-acetyl-1,3-diacryloylhexahydro-1,3,5-triazine; compounds having a reactive halogen described, for example, in U.S. Patent Nos. 3,288,775 and 2,732,303 and British Patent Nos. 974,723 and 1,167,207; N-hydroxymethylphthalimide; compounds having a reactive olefin described, for example, in U.S. Patent Nos. 3,635,718 and 3,232,763, British Patent No. 994,869, and Japanese Patent Application (OPI) Nos. 41221/1978 and 57257/1978; N-methylol compounds described, for example, in U.S. Patent Nos. 2,732,316 and 2,586,168; isocyanates described, for example, in U.S. Patent No. 3,103,437; aziridine compounds described, for example, in U.S. Patent No. 3,017,280 and 2,983,611 acid derivatives described, for example, in U.S. Patent Nos. 2,725,294 and 2,725,295; carbodiimide-type compounds described, for example, in U.S. Patent No. 3,100,704; epoxy-compounds described, for example, in U.S. Patent No. 3,091,537; halogenocarboxyaldehydes, such as mucochloric acid; dioxane derivatives, such as dihydroxydioxane, and dichlorodioxane; the above-mentioned dihydroquinoline-type compounds; compounds having a phosphorus-halogen bond, N-sulfonyloxyimide-type compounds; N-acyloxyimide-type compounds; isooxazole-type compounds described in U.S. Patent Nos. 3,321,313 and 3,543,292; N-carbamoylpyridinium salts; 2-sulfonyloxpyridinium salts or N-carbonyloxyimide-type compounds described in Japanese Patent Application (OPI) No. 43353/1981; or hardeners of inorganic compounds such as chrome alum and zirconium sulfate. The hardeners used in the present invention can also be used in combination with, instead of the above compounds, precursors for them, such as alkali metal bisulfite aldehyde adducts, methylol derivatives of hydantoin, primary aliphatic nitroalcohols, methyloxyethyl- sulfonyl-type compounds, and chloroethylsulfonyl-type compounds. When the present hardener is used in combination with another hardener, although the proportion of the present hardener used can be chosen depending on the purpose or desired effect, it is preferable that the proportion of the present hardener is 50 mol % or more.

In addition to the hardener used in the present invention, a compound that can facilitate the hardening of gelatin can also be used. Examples of such agents for facilitating hardening include nonprotonic solvents described in German Patent Application (OLS) No. 2,417,586, betain-type surface active agents described in Japanese Patent Application (OPI) No. 62045/1982, tertiary amines or their salts (e.g., those described, for example, in Japanese Patent Application (OPI) Nos. 1043/1981 and 9434/1986, German Patent Application (OLS) No. 2,138,305, and British Patent No. 1,284,305, and 1,269,983), various inorganic salts, and polyvalent alcohols. Naturally these agents for facilitating hardening can be used in combination with the present hardener plus the above-mentioned known hardener. For example, as an agent for facilitating hardening, a polymer containing a sulfinic acid group described in Japanese Patent Application (OPI) No. 4141/1981 can be additionally used in a system containing the present hardener and a vinylsulfonic-type hardener.

The gelatin to which the polymer coupler of the present invention will be applied may be any one of the so-called alkali-treated gelatins (lime-processed gelatins), obtained by immersion into an alkali bath before the extraction of gelatin during its production; acid-treated gelatin, obtained by immersion into an acid bath; double-immersion gelatin, obtained by immersion into an alkali bath and an acid bath; and enzyme- processed gelatin. Further, the hardener used in the present invention may be applied to gelatin having a low molecular weight obtained by heating the above gelatin in a water bath or allowing a proteolytic enzyme to act on the above gelatin, which action thereby partially hydrolyzes the gelatin.

Although it is advantageous to use gelatin, as a binder or a protective colloid that can be used in the emulsion layer or an intermediate layer of the present photographic material, other synthetic binders can also be used.

The silver halide emulsion of the color photographic material of this invention may be any type of halogen composition, including silver bromide, silver iodobromide, silver bromochloroiodide, silver chlorobromide, or silver chloride.

The silver halide grains of the silver halide emulsion may be regular grains comprising regular crystals such as cubes, octahedrons, or tetradecahedrons, or irregular crystals such as spherical crystals or platelike crystals, crystals having defects such as twin planes, or composites thereof.

The grain diameter of the silver halide may be fine grains about 0.2 _{/1}.m or less, or coarse grains wherein the diameter of the projected area is about 10 /1.m, and a polydisperse emulsion or a monodisperse emulsion can be used.

The silver halide photographic emulsions that can be used in this invention may be suitably prepared by known means, for example by the methods described in "I. Emulsion Preparation and Types" in Research Disclosure (RD), No. 17643 (December 1978), pp. 22-23, and in RD, No. 18716 (November 1979) p. 648; the methods described in P. Glafkides "Chemie et Phisique Photographique", Paul Montel (1967), in G.F. Duffin "Photographic Emulsion Chemistry", Focal Press (1966), and in V.L.Zelikman et al. "Making and Coating of Photographic Emulsion", Forcal Press (1964).

A monodisperse emulsion, as described in U.S. Patent Nos. 3,574,628 and 3,655,394, and in British Patent No. 1,413,748, is preferable.

Tabular grains having an aspect ratio of 5 or more can be used in the emulsion. Tabular grains can be easily prepared by the methods described in Gutoff "Photographic Science and Enggineering", Vol. 14, pp. 248-257 (1970), U.S. Patent Nos. 4,434,226, 4,414,310, 4,433,048, and 4,439,520, and British Patent No. 2,112,157.

The crystal structure of the emulsion grains may be uniform, the outer halogen composition of the crystal structure may be different from the inner halogen composition, or the crystal structure may be layered. Silver halides whose compositions are different may be joined by the epitaxial joint, or a silver halide may be joined, for example, to a compound other than silver halides, such as silver rhodanide or lead oxide.

Further, the silver halide may be a mixture of grains having various crystal shapes.

The silver halide emulsion may generally be physically ripened, chemically ripened, and spectrally sensitized. Additives that will be used in these steps are described in Research Disclosure No. 17643 and ibid. No. 18716, and the involved sections are listed in the Table below.

Known photographic additives that can be used in this invention are also described in the above- mentioned two Research Disclosures, and the involved sections are listed in the same Table below.

Various color couplers can be used in this invention, and typical examples are described in the patents in the above-mentioned Research Disclosure No. 17643, VII-C- G.

As yellow couplers, those described, for example, in U.S. Patent Nos. 3,933,501, 4,022,620, 4,326,024, and 4,401,752, Japanese Patent Publication No. 10739/1983, and British Patent Nos. 1,425,020 and 1,476,760 are preferable.

As magenta coupers, the 5-pyrazolone type and pyrazoloazole type are preferable, and those described in U.S. Patent Nos. 4,310,619 and 4,351,897, European Patent No. 73,636, U.S. Patent Nos. 3,061,432 and 3,725,067, Research Disclosure No. 24220 (June 1984), Japanese Patent Application (OPI) No. 33552/1985, Research Disclosure No. 24230 (1984), Japanese Patent Application (OPI) No. 43659/1985, and U.S. Patent Nos. 4,500,630 and 4,540,654 are more preferable.

The cyan couplers that can be used in this invention include phenol-type couplers and naphthol-type couplers, and those described in U.S. Patent Nos. 4,052,212, 4,146,396, 4,228,233, 4,296,200, 2,369,929, 2,801,171, 2,772,162, 2,895,826, 3,772,002, 3,758,308, 4,334,011, and 4,327,173, German Patent Application(OLS) No. 3,329,729,European Patent No. 121,365A, U.S. Patent Nos. 3,446,622, 4,333,999, 4,451,559, and 4,427,767, and European Patent No. 161,626A are more preferable.

As a colored coupler to rectify the unnecessary absorption of color-forming dyes, those couplers described in paragraph VII-G of Research Disclosure No. 17643, U.S. Patent No. 4,163,670, Japanese Patent Publication No. 39413/1982, U.S. Patent Nos. 4,004,929 and 4,138,258, and British Patent No. 1,146,368 can be preferably used in the present invention.

As a coupler which forms a dye having moderate diffusibility, those described in U.S. Patent No. 4,366,237, British Patent No. 2,125,570, European Patent No. 96,570, and German Patent Application (OLS) No. 3,234,533 are preferable.

Examples of a polymerized dye-forming coupler are described in U.S. Patent Nos. 3,451,820, 4,080,211, and 4,367,282, and British Patent No. 2,102,173.

A coupler that releases a photographically useful residue can be used in this invention. As a DIR coupler that releases a development retarder, those described in Japanese Patent Application (OPI) Nos. 151944/1982, 154234/1982, and 184248/1985, and U.S. Patent No. 4,248,962, which are cited in paragraph VII-F of the above-mentioned Research Disclosure No. 17643, are preferable.

As a coupler which releases, imagewise, a nucleating agent or a development accelerator upon developing, those described in British Patent Nos. 2,097,140, 2,131,188, and Japanese Patent Application (OPI) No. 157638/1984, and 170840/1984 are preferable.

Other couplers that can be incorporated in the photographic material of this invention include competitive couplers described in U.S. Patent No. 4,130,427, multi-equivalent couplers described in U.S. Patent Nos. 4,283,472, 4,338,393, and 4,310,618, DIR coupers which release a redox compound, as described in Japanese Patent Application (OPI) No. 185950/1985, and couplers which release a dye to regain a color after releasing, as described in European Patent No. 173,302A.

Couplers to be used in this invention may be incorporated in the photographic material by means of various known dispersion processes.

Examples of high boiling solvents for use in an oil-in-water type dispersion process are illustrated, for example, in U.S. Patent No. 2,322,027.

Processes and effects of the latex dispersion process and concrete examples of latices for impregnation are described, for example, in U.S. Patent No. 4,199,363 and German Patent Application (OLS) Nos. 2,541,274 and 2,541,230.

Adequate substrates that can be used in this invention are described, for example, on page 28 of the above-mentioned RD No. 17643, and on p. 647 (right column) to p. 648 (left column) of ibid. No. 18716.

The color photographic material according to this invention can be processed for development by conventional methods, such as described on pp. 28-29 of the abovementioned RD No. 17643 and on page 651 of ibid. No. 18716.

The silver halide color photographic material of the present invention is generally passed through a washing step and/or a stabilizing step after the desilvering process of fixing or bleach-fixing.

The amount of washing water in the washing step can be set in a wide range depending on the properties of the photographic material (due to the material used, for example, such as the couplers), the uses of the photographic material, the temperature of the washing water, the number of washing tanks (number of steps), the type of replenishing mode, such as counter-current mode or concurrent mode, as well as other conditions. The relationship between the number of washing tanks and the amount of water in the multistage counter-current mode can be determined according to a method described in Journal of the Society of Motion Picture and Television Engineers, Vol. 64, pp. 248-253 (May 1955). The number of steps of the multistage counter-current washing mode is preferably 2 to 6, more preferably 2 to 4.

With the multistage counter-current method the amount of washing water can be decreased considerably. However, bacteria propagate due to the increased time the water remains in the tanks, causing problems such as the adhesion of resulting suspended matter on the photographic material. To solve such problems in the method of processing of the present invention a color photographic material, a method of decreasing calcium and magnesium described in Japanese Patent Application No. 131632/1986 can be effectively used. Other agents that can be used include isothiazolone and cyabendazole compounds, described in Japanese Patent Application (OPI) No. 8542/1982, chlorine-type bactericides such as sodium chlorinated isocyanurate, benzotriazole, and other bactericides, described in Hiroshi Horiguchi Bokinbobai no Kagaku, Biseibutsu no Mekkin, Sakkin, Bobai Gijutsu, edited by Eiseigijutsu kai, and Bokinbobaizai Jiten, edited by Nihon Bokinbobai-gakkai.

The pH of the washing water for processing a photographic material acording to the present invention is 4 to 9, preferably 5 to 8. Although the temperature of the washing water and the period for washing are set differently according, for example, to the uses and properties of the photographic material, generally the temperature of the washing water and the period for washing are selected in the range of 15 to 45 ° C for 20 s, to 10 min, preferably 25 to 40 ° C for 30 s to 5 min.

Further, in the present invention a photographic material can be processed by using a stabilizing solution directly, instead of the above-mentioned washing water. In such a process of stabilizing, known methods are described, for example, in Japanese Patent Application (OPI) Nos. 8543/1982, 14834/1983, 184343/1984, 220345/1985, 238832/1985, 239784/1985, 239749/1985, 4054/1986, and 118749/1986. Particularly preferable for use is a stabilizing bath containing 1-hydroxyethylidene-1,1-diphosphonic acid, 5-chloro-2-methyl-4-isothiazoline-3-one, bismuth compounds or ammonium compounds.

In some cases a stabilizing process is carried out after the above-mentioned washing process, an example of which is a stabilizing bath containing formalin and a surface-active agent used as a final bath.

According to the silver halide color photographic material of the present invention, there are attained a superior fastness to diffusion of the employed couplers, a good color reproduction and a high level color-forming property. Further, according to the invention, there are attained a rapid hardening-reaction of gelatin and less posthardening of the film not to soften by swelling even in the rapid and higher-temperature processing over normal temperature to afford a photograph having an excellent preservability.

In addition the silver halide color photographic material of the present invention can afford a photograph with a remarkably inproved sharpness of an image because of high film-strength so as to make the coating layers thinner.

Next, the present invention will be described in detail in accordance with examples.

### Example 1

A color photographic material (Sample 101) consisting of layers of the following composition was prepared on an undercoated triacetate cellulose film base.

### (Composition of photosensitive layers)

In the following compositions, the coating amount of silver halide and colloidal silver are each indicated in g/m² in terms of silver, the coating amount of the coupler, additive and gelatin are each indicated in g/m², and the coating amount of the sensitizing dye is indicated in mol per mol of silver halide in the same layer.

A surface-active agent was added to each layer as a coating aid.

### Preparation of Samples 102 - 116

Samples 102 to 116 were prepared by repeating the same procedure as Sample 101, except that the coupler E-1 and the hardener HT-1 in Sample 101 were changed to those shown respectively in Table 1. In all samples, a high boiling organic solvent was not used.

On the other hand, in order to determine the film strength of the respective emulsion layers, samples corresponding to Samples 101 to 116 but not containing the second layer (protective layer) were prepared, and the Vickers hardness of each thus-prepared sample was measured by a Terasawa's micro-hardness tester (MM-2 type) (using a Knoop indenter). Vickers hardness is described in D. Talor "The Physical Meaning of Indentation and Scratch. Hardness.", British Journal of Applied Physics Vol. 7 p. 260 (1956).

In the preparation of Samples 101 to 116, the oil-soluble coupler (E-1 or E-2) was heated and dissolved in ethyl acetate of an 8-times amount by weight of the coupler. The resulting solution was then mixed with an 8% gelatin aqueous solution (2 times the volume of the coupler solution) containing a surface-active agent W-1, and it was emulsified by a homogenizer. After removing ethyl acetate from the thus-prepared emulsion, it was added to the coating solution. The water-soluble polymer coupler was dissolved in water so as to be a 5 wt. percent solution, and it was then added to the coating solution. The coating amount for Samples 101 to 116 was the same.

The constitution of the materials used are shown below.

Each of Samples 101 to 116 was subjected to a light exposure of an Wolfram light source at a color temperature of 4,800 ° K through a filter so that the maximum exposure amount was 25 CMS, and it was then subjected to development processing at 38 ° C according to the following process (I).

The composition of each processing solution was as follows:

A density measurement was conducted on each of the thus-processed samples, and the highest density was shown as Dᵢ.

Further, color photographic materials (Samples 101' - 116') were prepared by repeating the same procedure as in Samples 101 - 116, except that the composition of the multi-layers was changed as hereinbelow described. These samples were subjected to the same exposure of light and then the same development processing as Samples 101 - 116. A density measurement was conducted on each of the thus-processed samples, and the highest density was shown as D₂. The value D₂/Di is indicative of the fastness to diffusion.

### (Composition of photosensitive layers)

In the following compositions, each ingredient is indicated as in Sample 101.

In each layer a surface-active agent was added as a coating aid.

The results are shown in Table 1.

Although the water soluble polymer coupler is excellent in film strength as compared to the oil soluble coupler, the degree of diffusion to the other layer is large, as shown in the data of the comparative sample.

In contrast with this, as in the present invention (Samples 111 to 116), when using the hardener acting by activation of the water soluble polymer containing a non-color-forming repeating unit having a carboxyl group and with activation of the carboxyl group, the film strength is excellent and the color-developing property is improved by restraining the diffusion of the coupler to the other layers.

### Example 2

A color photographic material (Sample 201) was prepared by multi-coatings composed of the following composition on an undercoated triacetate cellulose film base.

### (Composition of photosensitive layers)

In the following compositions, each ingredient is indicated as in Example 1.

In each layer described above, a surface-active agent was added as a coating aid. The structural formula or chemical name of the compound used in this Example are shown below.
Oil - 1 Tricresyl phosphate
Oil - 2 Dibutyl phthalate
Oil - 3 Bis(2-ethylhexyl)phthalate
HT-1

### Preparation of Samples 202 to 209

The same procedure as for Sample 201 was repeated, except that the coupler E-1 in the 11th layer and the 12th layer and the hardener HT-1 in the 14th layer were changed to those shown in Table 2 at equal molar ratios, thus preparing Samples 202 to 209. These samples were each subjected to an exposure of green light through a wedge and then to development processing according to the following processing process (II).

The density of each thus-processed sample was measured, and the density of yellow at the magenta color-forming layer was evaluated as a criterion for coupler diffusion from the blue-sensitive layer to the green-sensitive layer.

The composition of each processing solution was as follows:
Color developing solution

Same as processing process (I).

The thus-obtained samples according to the present invention were all of excellent film strength. As is apparent from the results in Table 2, the diffusion of couplers to other layers of samples of the present invention is restrained to such a degree as to present no practical problem.

### Example 3

A color photographic material was prepared by multi-coatings composed of the following composition on an undercoated triacetate cellulose film base as Sample 301.

In each layer described above, a gelatin hardener HT-1 (Same as in Example 1) and a surfactant were added.

The compounds used in the above layers were as follows:

The high-boiling organic solvents Oil-1 and Oil-2 are the same as in Example 2.

The emulsion grains used in the 10th layer and 11th layer of Sample 301 are both plate-twin type, having an aspect ratio of 8.

### Preparation of Samples 302 to 310

The same procedure as for Sample 301 was repeated, except that the coupler F-6 in the 10th layer and the 11th layer and the film hardener HT-1 in the 13th layer were changed to those shown in Table 3, thus preparing Samples 302 to 310. Each of Samples 301 to 310 were subjected to an exposure of white light through a wedge and then to processing as described below.

The same density measurement as in Example 2 was conducted on each of the thus-processed samples, and the results are shown in Table 3. The samples according to the present invention were of excellent film strength, and as is apparent from the results in this Table, the diffusion of couplers to other layers of these samples are restrained to such a level as to present no practical problem.

The composition of each processing solution was as follows:

### Example 4

Samples 401 to 416 were prepared by repeating the same procedure as in Example 1, except that the polymer couplers were changed to those shown in Table 4.

The thus-prepared samples were subjected to the same treatments as in Example 1 and then the same measurements as in Example 1 were conducted.

The results are shown in Table 4.

As is evident from the results in Table 4, when using the coupler of the present invention (Samples 411 to 416), the film strength is excellent and the color-forming property is improved by restraining the diffusion of coupler to the other layers.

### Example 5

Samples 501 to 509 were prepared by repeating the same procedure as in Example 2, except that the polymer couplers were changed to those shown in Table 5.

The thus-prepared Samples were subjected to the same treatments as in Example 2 and then the same measurements as in Example 2 were conducted.

The results are shown in Table 5.

The thus-obtained samples according to the present invention (Samples 506 to 509) were all of excellent film strength. As is apparent from the results in Table 5, the diffusion of couplers to other layers of samples of the present invention is restrained to such a degree as to present no practical problem.

### Example 6

Samples 601 to 610 were prepared by repeating the same procedure as in Example 3, except that the polymer couplers were changed to those shown in Table 6.

The thus-prepared samples were subjected to the same treatments as in Example 3 and then the same measurements as in Example 3 were conducted.

The results are shown in Table 6.

The samples according to the present invention (Samples 606 to 610) were of excellent film strength, and as is apparent from the results in Table 6, diffusion of couplers to other layers of these samples are restrained to such a level as to present no practical problem.

## Claims

1. A silver halide color photographic material which comprises a hardener that acts by activating a carboxyl group and at least one polymer coupler comprising at least one repeating unit of the following formula (I): wherein A represents a vinyl polymer unit having a color coupler residue capable of coupling with the oxidized product of an aromatic primary amine developing agent, characterized in that said polymer coupler further has at least one repeating unit of the following formula (II): wherein B represents a vinyl monomer unit having at least one group selected from an amino group and -COOM, wherein M represents a hydrogen atom, an alkali metal or ammonium, and that said polymer coupler is water-soluble.

The silver halide color photographic material of claim 1, wherein the monomer unit represented by formula (I) capable of coupling with the oxidized product of an aromatic primary amine developing agent to form a dye is represented by formula (III):
wherein R represents a hydrogen atom, a chlorine atom, or an alkyl group having 1 to 4 carbon atoms; D represents -COO-, -CONR'-, or a substituted or unsubstituted phenyl group; E represents a substituted or unsubstituted alkylene group, phenylene group, or aralkylene group; F represents -CONR'-, -NR'CONR'-, -NR'COO-, -NR'CO-, -OCONR'-, -NR'-, -COO-, -OCO-, -CO-, -0-, -S0₂-, -NR'S0₂-, or -S0₂NR'-, in which R' represents a hydrogen atom or a substituted or unsubstituted alkyl group or aryl group, and if two or more R' are in the same molecule, they may be the same or different;
î, m, and n are 0 or 1, provided that ℓ , m, and n are not 0 at the same time, and Q represents a cyan, magenta, or yellow dye-forming coupler residue capable of coupling with the oxidized product of an aromatic primary amine developing agent to form a dye.
The silver halide color photographic material of claim 2, wherein the color coupler residue represented by Q is selected from a residue represented by the phenol type (IV) or (V), or the naphthol type (VI) or (VII) (a hydrogen atom other than one positioned at the coupling position or the 1-positioned OH group will split off to join with F of formula (III))
wherein R¹¹ represents a group capable of substitution onto a phenol ring or a naphthol ring;
R¹² represents -CONR¹³R¹⁴, -NHCOR¹³, -NHCOOR¹⁵, -NHSO₂R¹⁵, -NYCONR¹³R¹⁴, or -NHSO₂R¹³R¹⁴, in which R¹³ or R¹⁴ represents a hydrogen atom, an aliphatic group, an aromatic group, a heterocyclic group, R¹⁵ represents an aliphatic group, an aromatic group, or a heterocyclic group, R¹³ and R¹⁴ may bond together to form a heterocyclic ring;
p' is an integer of 0 to 3, q' is an integer of 0 to 2, r' and s' are each integers of 0 to 4;
X represents an oxygen atom, a sulfur atom, or R¹⁶ N , in which R¹⁶ represents a hydrogen atom or a monovalent substituent;
Z represents a hydrogen atom, or a group that can split off by the coupling reaction; and
Y represents a group of atoms required to form a 5-, 6- or 7-membered ring together with the carbon atom.

4. The silver halide color photographic material of claim 2, wherein the color forming coupler residue represented by Q is selected from a residue represented by the following formulae (VII), (VIII), (IX), (X), (XI), (XII), and (XIII), and they are connected to F of formula (III) at a part of Ar, Z², and R²⁰ to R³²
wherein Ar represents a substituent capable of substitution at the first position of a 2-pyrazoline-5- on coupler;
R²⁰ represents an unsubstituted or substituted anilino group, an unsubstituted or substituted acylamino group, or an unsubstituted or substituted ureido group;
R²¹, R²², R²³, R²⁴, R²⁵, R²⁶, R²⁷, R²⁸, R²⁹, R³⁰, R³¹ and R³² each represent a hydrogen atom, a hydroxyl group, an unsubstituted or substituted alkyl group, an unsubstituted or substituted aryl group, an unsubstituted or substituted heterocyclic group; an alkylamino group, an acylamino group, an anilino group, an alkoxycarbonyl group, an alkylcarbonyl group, arylcarbonyl group, an alkylthio group, an arylthio group, a carbamoyl group, a sulfamoyl group, or a sulfonamido group; and
Z² represents a hydrogen atom or a group which can split-off by a coupling-reaction.

5. The silver halide color photographic material of claim 2, wherein the color coupler residue represented by Q is selected from a pivaloylacetoanilido type (XIV), or a benzoylacetoanilido type (XV) or (XVI)
wherein R³³, R³⁴, R35, and R³⁶, which may be the same or different, each represent a hydrogen atom or a substituent of the residue of a yellow color-forming coupler, and
Z³ represents a hydrogen atom or a group that can split off by a coupling reaction. The silver halide color photographic material as claimed in Claim 1, wherein the monomer unit represented by formula (II) is selected from a unit represented by the following formula (XXIVa) or (XXIVb):
wherein R⁴⁵ represents a hydrogen atom, a lower alkyl group having 1 to 4 carbon atoms, or a chlorine atom; P represents -COO-, -CONHR46'-, or a substituted or unsubstituted phenylene group; T represents -COO-, -CONH-, or a substituted or unsubstituted phenylene group; L represents a substituted or unsubstituted alkylene, a phenylene or an aralkylene group; M represents a hydrogen atom, an alkali metal or ammonium; m' and n' each represent 0 or 1; and R⁴⁶ and R^{46,} each represent a hydrogen atom, or a substituted or unsubstituted alkyl or aryl group.

7. The silver halide color photographic material of claim 1, wherein the water-soluble polymer coupler contains a non-color-forming ethylenically-unsaturated monomer unit which does not undergo a coupling reaction with the oxidation product of an aromatic primary amine developing agent other than those represented by formulas (I) and (II), and which does not contain -COOM or an amino group in the molecule in an amount of 60% or less in terms of the total of the monomer units represented by formulas (I) and (II).

8. The silver halide color photographic material of claim 7, wherein the non-color-forming ethylenically-unsaturated monomer unit other than the ones represented by formulae (I) and (II) is selected from acrylate esters, methacrylate esters, crotonate esters, vinyl esters, maleate diesters, fumarate diesters, itaconate diesters, acrylamides, methacrylamides, vinyl ethers, and styrenes.

9. The silver halide color photographic material of claim 1, wherein the proportion of the color forming moiety corresponding formula (I) in the polymer coupler is 5 to 80 wt.%.

10. The silver halide color photographic material of claim 1, wherein the proportion of the component (monomer unit) corresponding to formula (II) in the polymer coupler is 20 to 95 wt.%.

11. The silver halide color photographic material of claim 1, wherein the polymer coupler is added in an amount of 0.005 to 0.5 mol, per mol of silver, in terms of the coupler monomer unit represented by formula (I).

12. The silver halide color photographic material of claim 1, wherein the molecular weight of the polymer coupler is 5 x 10³ to 1 x 10⁷.

13. The silver halide color photographic material of claim 1, wherein the molecular weight equivalent of the polymer coupler is about 250 to 4000.

14. The silver halide color photographic material of claim 1, wherein the hardener is selected from compounds represented by the following formula (XXV):
wherein R⁴⁷ and R⁴⁸, which may be the same or different, each represent an alkyl group, an aryl group, or an aralkyl group in which R⁴⁷ and R⁴⁸ may bond together with the nitrogen atom to form a heterocyclic ring, R⁴⁹ represents a substituent such as a hydrogen atom, a halogen atom, a carbamoyl group, a sulfo group, a ureido group, an alkoxy group and an alkyl group, and X^{e} represents an anion and becomes a counter ion to the N-carbamoylpyridinium salt.

15. The silver halide color photographic material of claim 1, wherein the hardener is selected from compounds represented by the following formula (XXVI):
wherein R⁴⁷ and R⁴⁸, which may be the same or different, each represent an alkyl group, an aryl group, or an aralkyl group in which R⁴⁷ and R⁴⁸ may bond together with the nitrogen atom to form a heterocyclic ring, R⁴⁹ represents a substituent such as a hydrogen atom, a halogen atom, a carbamoyl group, a sulfo group, a ureido group, an alkoxy group and an alkyl group, and X^{e} represents an anion and becomes a counter ion to the N-carbamoylpyridinium salt.

16. The silver halide color photographic material of claim 1, wherein the hardener is selected from compounds represented by the following formula (XXVII):
wherein R⁵⁰, R⁵¹, R⁵², and R⁵³, which may be the same or different, each represent an alkyl group, an aralkyl or an aryl group, in which R⁵⁰, R⁵¹, R⁵², and R⁵³ may bond together to form a ring,
X represents a group that can split off when the compound represented by formula (XXVII) reacts with a nucleophilic reagent, and
Y^{e} represents an anion, and if Y^{e} represents a sulfonate ion, it may bond to X, R⁵⁰, R⁵¹, R⁵² or R⁵³ to form an inner salt.

17. The silver halide color photographic material of claim 1, wherein the hardener is selected from compounds represented by the following formula (XXVIII): wherein R⁵⁴ represents an alkyl group, a cycloalkyl group, an alkoxyalkyl group, or an aralkyl group; R⁵⁴' represents a group as defined for R⁵⁴, or wherein R⁵⁵ represents an alkylene group; R⁵⁶ and R⁵⁷, which may be the same or different, each represent an alkyl group (R⁵⁶ and R⁵⁷ may bond together with the nitrogen atom to form a heterocyclic ring); R⁵⁸ represents an alkyl group; X^{e} represents an anion, and if R⁵⁸ is substituted by a sulfo group, an inner salt is formed.

18. The silver halide color photographic material of claim 1, wherein the hardener is selected from compounds represented by the following formula (XXIX):
wherein R⁵⁹ represents an alkyl group, an aryl group or an aralkyl group, R⁶⁰ and R⁶¹, which may be the same or different, each represent a substituent, (R⁶⁰ and R⁶¹ may bond together with the pyridinium ring skeleton to form a condensed ring),
X represents a group that can split off when the compounds represented by formula (XXIX) react with a nucleophilic reagent, and
Y^{e} represents an anion, and if R⁵⁹ is substituted by a sulfo group, an inner salt is formed.

19. The silver halide color photographic material of claim 1, wherein the hardener is selected from compounds represented by the following formula (XXX):
wherein R⁶³ and R⁶⁴, which may be the same or different, each represent an alkyl group, an aryl group, or an aralkyl in which R⁶³ and R⁶⁴ may bond together with the nitrogen atom to form a heterocyclic ring, R⁶⁵ represents an alkyl group, an aryl group, or an aralkyl group, and X^{e} represents an anion.

20. The silver halide color photographic material of claim 1, wherein the hardener is selected from compounds represented by the following formula (XXXI):
wherein R⁶⁶ represents a straight-chain or branched alkyl group, an aralkyl group, an aryl group, an alkenyl group, or a heteroaromatic group, and X represents a group that can split off when the compounds represented by formula (XXXI) react with a nucleophilic reagent.

21. The silver halide color photographic material of claim 1, wherein the hardener is selected from compounds represented by the following formula (XXXII):
wherein R⁶⁹ and R⁷⁰ represent a straight-chain or branched alkyl group, a cycloalkyl group, an aralkyl group, an aryl group, an alkenyl group, or a heterocyclic group, R⁶⁹ and R⁷⁰ may bond together to form a heterocyclic ring;
R⁷¹ represents a straight-chain or branched alkyl group, a cycloalkyl group, an aralkyl group, an aryl group, an alkenyl group, a heterocyclic group, or a group in which R⁷² and R⁷³ represent a straight-chain or branched alkyl group, an aralkyl group, an aryl group, or an alkenyl group,
R⁶⁹ and R⁷⁰ or R⁷² and R⁷³ may bond together with the nitrogen atom to form a ring, and
X represents a group that can split off when the compounds represented by formula (XXXII) react with a nucleophilic reagent.

22. The silver halide color photographic material of claim 1, wherein the hardener is selected from compounds represented by the following formula (XXXIII):
wherein R⁷⁴, R⁷⁵, R⁷⁶, R⁷⁷, R⁷⁸, and R⁷⁹, which may be the same or different, each represent a straight-chain or branched alkyl group, an aralkyl group, or an aryl group (R⁷⁴, R⁷⁵, R⁷⁶, R⁷⁷, R⁷⁸, and R⁷⁹ may bond together to form a ring),
X represents a group that can split off when the compounds represented by formula (XXXIII) react with a nucleophilic reagent, and
Y^{e} represents an anion.

## Patentansprüche

1. Farbfotografisches Silberhalogenidmaterial, das einen Härter umfaßt, der durch Aktivierung einer Carboxylgruppe und mindestens eines Polymerkupplers wirkt und der mindestens eine sich wiederholende Einheit der folgenden Formel (I) aufweist: worin A eine Vinylpolymereinheit mit einem Farbkupplerrest darstellt, der mit dem oxidierten Produkt eines aromatischen primären Aminentwicklungsmittels kuppeln kann, dadurch gekennzeichnet, daß der Polymerkuppler außerdem mindestens eine sich wiederholende Einheit der folgenden Formel (11) besitzt: worin B eine Vinylmonomereinheit mit mindestens einer Gruppe, gewählt aus einer Aminogruppe und -COOM bedeutet, worin M ein Wasserstoffatom, ein Alkalimetall oder Ammonium bedeutet, und der Polymerkuppler wasserlöslich ist.

2. Farbfotografisches Silberhalogenidmaterial nach Anspruch 1, worin die durch Formel (I) dargestellte Monomereinheit mit dem oxidierten Produkt eines aromatischen primären Aminentwicklungsmittels kuppeln kann, um einen Farbstoff zu bilden, der durch die Formel (111) dargestellt wird: worin R ein Wasserstoffatom, ein Chloratom oder eine Alkylgruppe mit 1 bis 4 Kohlenstoffatomen bedeutet; D -COO-, -CONR'- oder eine substituierte oder unsubstituierte Phenylgruppe bedeutet; E eine substituierte oder unsubstituierte Alkylengruppe, Phenylengruppe oder Aralkylengruppe bedeutet; F -CONR'-, -NR'CONR'-, -NR'COO-, -NR'CO-, -OCONR'-, -NR'-, -COO-, -OCO-, -CO-, -O-, -NR'S0₂- oder -S0₂NR'-, bedeutet, in denen R' ein Wasserstoffatom oder eine substitierte oder unsubstituierte Alkylgruppe oder Arylgruppe bedeutet, und wenn zwei oder mehrere R' in demselben Molekül vorliegen, diese gleich oder verschieden sein können; I, m, und n 0 oder 1 sind, unter der Voraussetzung, daß I, m und n nicht gleichzeitig 0 sind und Q einen Cyan-, Magenta- oder einen gelben Farbstoff bildenden Kupplerrest bedeutet, der mit dem oxidierten Produkt eines aromatischen primären Entwicklungsmittels kuppeln kann, um einen Farbstoff zu bilden.

3. Farbfotografisches Silberhalogenidmaterial nach Anspruch 2, worin der durch Q dargestellte Farbkupplerrest gewählt ist aus einem Rest, dargestellt von dem Phenoltyp (IV) oder (V) oder dem Naphtholtyp (VI) oder (VII) (ein anderes Wasserstoffatom als das an der Kupplerposition oder der OH-Gruppe in 1-Stellung wird abgespalten, um an F der Formel (111) zu binden): worin R¹¹ eine Gruppe bedeutet, die an einen Phenolring oder Naphtholring substituiert sein kann; R¹² -CONR^{I3}R¹⁴, -NHCOR¹³, -NHCOOR¹⁵, -NHS0₂R¹⁵, -NYCONR¹³R¹⁴ oder -NHS0₂R¹³R¹⁴ bedeutet, in denen R¹³ oder R¹⁴ ein Wasserstoffatom, eine aliphatische Gruppe, eine aromatische Gruppe oder eine heterocyclische Gruppe bedeutet, R¹⁵ eine aliphatische Gruppe, eine aromatische Gruppe oder eine heterocyclische Gruppe bedeutet, R¹³ und R¹⁴ miteinander verbunden sein können, um einen heterocyclischen Ring zu bilden;
p' eine ganze Zahl von 0 bis 3 ist, q' eine ganze Zahl von 0 bis 2 ist, r' und s' jeweils ganze Zahlen von 0 bis 4 sind;
X ein Sauerstoffatom, ein Schwefelatom oder R¹⁶ N bedeutet, worin R¹⁶ ein Wasserstoffatom oder einen monovalenten Substituenten bedeutet;
Z ein Wasserstoffatom oder eine Gruppe bedeutet, die bei der Kupplungsreaktion abgespalten werden kann; und
Y eine Gruppe von Atomen bedeutet, die erforderlich ist, um einen 5-, 6-, oder 7-gliedrigen Ring zusammen mit dem Kohlenstoffatom zu bilden.

4. Farbfotografisches Silberhalogenidmaterial nach Anspruch 2, worin der durch Q dargestellte farbbildende Kupplerrest gewählt ist aus einem Rest, dargestellt durch die folgenden Formeln (VII), (VIII), (IX), (X), (XI) (XII) und (XIII), und diese an F der Formel (III) an einem Teil von Ar, Z² und R²⁰ bis R³² gebunden sind, worin Ar einen Substituenten bedeutet, der an der ersten Position eines 2-Pyrazolin-5-on-Kupplers substituieren kann;
R²⁰ eine unsubstituierte oder substituierte Anilinogruppe, eine unsubstituierte oder substituierte Acylaminogruppe oder eine unsubstituierte oder substituierte Ureidogruppe bedeutet;
R²¹, R²², R²³, R²⁴, R²⁵, R²⁶, R²⁷, R²⁸, R²⁹, R³⁰, R³¹ und R³² jeweils ein Wasserstoffatom, eine Hydroxylgruppe, eine unsubstituierte oder substituierte Alkylgruppe, eine unsubstituierte oder substituierte Arylgruppe, eine unsubstituierte oder substituierte heterocyclische Gruppe, eine Alkylaminogruppe, eine Acylaminogruppe, eine Anilinogruppe, eine Alkoxycarbonylgruppe, eine Alkylcarbonylgruppe, eine Arylcarbonylgruppe, eine Alkylthiogruppe eine Arylthiogruppe, eine Carbamoylgruppe, eine Sulfamoylgruppe oder eine Sulfonamidogruppe bedeuten; und
Z² ein Wasserstoffatom oder eine Gruppe bedeutet, die bei der Kupplungsreaktion abgespalten werden kann.

5. Farbfotografisches Silberhalogenidmaterial nach Anspruch 2, worin der durch Q dargestellte Farbkupplerrest gewählt ist aus einem Pivaloylacetoanilidotyp (XIV) oder einem Benzoylacetonalididotyp (XV) oder (XVI) worin R³³, R³⁴, R³⁵ und R³⁶, die gleich oder verschieden sein können, jeweils ein Wasserstoffatom oder einen Substituenten des Restes eines eine gelbe Farbe bildenden Kupplers bedeuten und Z³ ein Wasserstoffatom oder eine Gruppe bedeutet, die durch eine Kupplungsreaktion abgespalten werden kann.

6. Farbfotografisches Silberhalogenidmaterial nach Anspruch 1, worin die durch Formel (11) dargestellte Monomereinheit gewählt ist aus einer Einheit, dargestellt durch die folgende Formel (XXIVa) oder (XXIVb): worin R⁴⁵ ein Wasserstoffatom, eine niedrige Alkylgruppe mit 1 bis 4 Kohlenstoffatomen oder ein Chloratom bedeutet; P -COO-, -CONHR⁴⁶- oder eine substituierte oder unsubstituierte Phenylengruppe bedeutet; T -COO-, -CONH- oder eine substituierte oder unsubstituierte Phenylengruppe bedeutet; L eine substituierte oder unsubstituierte Alkylengruppe, eine Phenylengruppe oder eine Aralkylengruppe bedeutet; M ein Wasserstoffatom, ein Alkalimetall oder Ammonium bedeutet; m' und n' jeweils 0 oder 1 bedeuten; und R⁴⁶ und R⁴⁶' jeweils ein Wasserstoffatom oder eine substituierte oder unsubstituierte Alkylgruppe oder Arylgruppe bedeuten.

7. Farbfotografisches Silberhalogenidmaterial nach Anspruch 1, worin der wasserlösliche Polymerkuppler eine nichtfarbbildende ethylenisch ungesättigte Monomereinheit enthält, die mit keinem anderen Oxidationsprodukt eines aromatischen primären Aminentwicklungsmittels als mit denen, durch die Formeln (I) und (11) dargestellten, eine Kupplungsreaktion eingeht, und die keine -COOM oder Aminogruppe in dem Molekül in einer Menge von 60% oder weniger, ausgedrückt als die Gesamtzahl der Monomereinheiten, dargestellt durch die Formeln (I) und (11), enthält.

8. Farbfotografisches Silberhalogenidmaterial nach Anspruch 7, worin die nichtfarbbildende ethylenisch ungesättigte Monomereinheit außer den durch die Formeln (I) und (11) dargestellten, gewählt ist aus Acrylatestern, Methacrylatestern, Crotonatestern, Vinylestern, Maleatdiestern, Fumaratdiestern, Itaconatdiestern, Acrylamiden, Methacrylamiden, Vinylethern und Styrolen.

9. Farbfotografisches Silberhalogenidmaterial nach Anspruch 1, worin der Anteil des farbbildenden Restes entsprechend Formel (I) in dem Polymerkuppler 5 bis 80 Gew.-% beträgt.

10. Farbfotografisches Silberhalogenidmaterial nach Anspruch 1, worin der Anteil der Komponente (Monomereinheit) entsprechend Formel (11) im dem Polymerkuppler 20 bis 95 Gew.-% beträgt.

11. Farbfotografisches Silberhalogenidmaterial nach Anspruch 1, worin der Polymerkuppler in einer Menge von 0.005 bis 0,5 mol pro mol Silber, ausgedrückt als die Kupplermonomereinheit, dargestellt durch Formel (I), zugegeben wird.

12. Farbfotografisches Silberhalogenidmaterial nach Anspruch 1, worin das Molekulargewicht des Polymerkupplers 5 x 10³ bis 1 x 10⁷ beträgt.

13. Farbfotografisches Silberhalogenidmaterial nach Anspruch 1, worin das Molekulargewichtsäquivalent des Polymerkupplers etwa 250 bis 4000 beträgt.

14. Farbfotografisches Silberhalogenidmaterial nach Anspruch 1, worin der Härter gewählt ist aus Verbindungen, dargestellt durch die folgende Formel (XXV): worin R⁴⁷ und R⁴⁸, die gleich oder verschieden sein können, jeweils eine Alkylgruppe, eine Arylgruppe oder eine Aralkylgruppe bedeuten, in denen R⁴⁷ und R⁴⁸ miteinander mit dem Stickstoffatom verbunden sein können, um einen heterocyclischen Ring zu bilden, R⁴⁹ einen Substituenten, wie ein Wasserstoffatom, ein Halogenatom, eine Carbamoylgruppe, eine Sulfogruppe, eine Ureidogruppe, eine Alkoxygruppe und eine Alkylgruppe, bedeutet und X^{e} ein Anion bedeutet und ein Gegenion zu dem N-Carbamoylpyridiniumsalz wird.

15. Farbfotografisches Silberhalogenidmaterial nach Anspruch 1, worin der Härter gewählt ist aus Verbindungen, dargestellt durch die folgende Formel (XXVI): worin R⁴⁷ und R⁴⁸, die gleich oder verschieden sein können, jeweils eine Alkylgruppe, eine Arylgruppe oder eine Aralkylgruppe bedeuten, in denen R⁴⁷ und R⁴⁸ miteinander mit dem Stickstoffatom verbunden sein können, um einen heterocyclischen Ring zu bilden, R⁴⁹ einen Substituenten, wie ein Wasserstoffatom, ein Halogenatom, eine Carbamoylgruppe, eine Sulfogruppe, eine Ureidogruppe, eine Alkoxygruppe und eine Alkylgruppe bedeutet, und X^{e} ein Anion bedeutet und ein Gegenion zu dem N-Carbamoylpyridiniumsalz wird.

16. Farbfotografisches Silberhalogenidmaterial nach Anspruch 1, worin der Härter gewählt ist aus Verbindungen, dargestellt durch die folgende Formel (XXVII): worin R⁵⁰, R⁵¹, R⁵² und R⁵³, die gleich oder verschieden sein können, jeweils eine Alkylgruppe, eine Aralkylgruppe oder eine Arylgruppe bedeuten, in den R⁵⁰, R⁵¹, R⁵² und R⁵³ miteinander verbunden sein können, um einen Ring zu bilden,
X eine Gruppe bedeutet, die abgespalten werden kann, wenn die durch die Formel (XXVII) dargestellte Verbindung mit einem nukleophilen Reagens reagiert und
Y^{e} ein Anion bedeutet und, wenn Y^{e} ein ein Sulfonatanion bedeutet, es an X, R⁵⁰, R⁵¹, R⁵² oder R⁵³ gebunden sein kann, um ein inneres Salz zu bilden.

17. Farbfotografisches Silberhalogenidmaterial nach Anspruch 1, worin der Härter gewählt ist aus Verbindungen, dargestellt durch die folgende Formel (XXVIII):
_{R}54-_{N} = N-R⁵⁴' (XXVIII)
worin R⁵⁴ eine Alkylgruppe, eine Cycloalkylgruppe, eine Alkoxyalkylgruppe oder eine Aralkylgruppe bedeutet,
R⁵⁴' eine Gruppe bedeutet, wie für R⁵⁴ definiert oder worin R⁵⁵ eine Alkylengruppe bedeutet; R⁵⁶ und R⁵⁷, die gleich oder verschieden sein können, jeweils eine Alkylgruppe bedeuten (R⁵⁶ und R⁵⁷ können miteinander mit dem Stickstoffatom verbunden sein, um einen heterocyclischen Ring zu bilden); R⁵⁸ eine Alkylgruppe bedeutet; X^{e} ein Anion bedeutet, und, wenn R⁵⁸ mit einer Sulfogruppe substituiert ist, ein inneres Salz gebildet wird.

18. Farbfotografisches Silberhalogenidmaterial nach Anspruch 1, worin der Härter gewählt ist aus Verbindungen der folgenden Formel (XXIX): worin R⁵⁹ eine Alkylgruppe, eine Arylgruppe oder eine Aralkylgruppe bedeutet, R⁶⁰ und R⁶¹, die gleich oder verschieden sein können, jeweils einen Substituenten bedeuten (R⁶⁰ und R⁶¹ können zusammen mit dem Pyridiniumringskelett verbunden sein, um einen kondensierten Ring zu bilden),
X eine Gruppe bedeutet, die abgespalten werden kann, wenn die durch die Formel (XXIX) dargestellten Verbindungen mit einem nukleophilen Reagens reagieren und
Y^{e} ein Anion bedeutet, und wenn R⁵⁹ mit einer Sulfogruppe substituiert ist, ein inneres Salz gebildet wird.

19. Farbfotografisches Silberhalogenidmaterial nach Anspruch 1, worin der Härter gewählt ist aus Verbindungen, dargestellt durch die folgende Formel (XXX): worin R⁶³ und R⁶⁴, welche gleich oder verschieden sein können, jeweils eine Alkylgruppe, eine Arylgruppe oder eine Aralkylgruppe bedeuten, in denen R⁶³ und R⁶⁴ zusammen mit dem Stickstoffatom verbunden sein können, um einen heterocyclischen Ring zu bilden, R⁶⁵ eine Alkylgruppe, eine Arylgruppe oder eine Aralkylgruppe bedeutet, und X^{e} ein Anion bedeutet.

20. Farbfotografisches Silberhalogenidmaterial nach Anspruch 1, worin der Härter gewählt ist aus Verbindungen, dargestellt durch die folgende Formel (XXXI) worin R⁶⁶ eine geradkettige oder verzweigte Alkylgruppe, eine Aralkylgruppe, eine Arylgruppe, eine Alkenylgruppe oder eine heteroaromatische Gruppe bedeutet, und X eine Gruppe bedeutet, die abgespalten werden kann, wenn die durch die Formel (XXXI) dargestellten Verbindungen mit einem nukleophilen Reagens reagieren.

21. Farbfotografisches Silberhalogenidmaterial nach Anspruch 1, worin der Härter gewählt ist aus Verbindungen, dargestellt durch die folgende Formel (XXXII): worin R⁶⁹ und R⁷⁰ eine geradkettige oder verzweigte Alkylgruppe, eine Cycloalkylgruppe, eine Aralkylgruppe, eine Arylgruppe, eine Alkenylgruppe oder eine heterocyclische Gruppe bedeuten, R⁶⁹ und R⁷⁰ miteinander verbunden sein können, um einen heterocyclischen Ring zu bilden;
R⁷¹ eine geradkettige oder verzweigte Alkylgruppe, eine Cycloalkylgruppe, eine Aralkylgruppe, eine Arylgruppe, eine Alkenylgruppe, eine heterocyclische Gruppe oder eine Gruppe bedeutet, in der R⁷² und R⁷³ eine geradkettige oder verzweigte Alkylgruppe, eine Aralkylgrupe, eine Arylgruppe oder eine Alkenylgruppe bedeuten,
R⁶⁹ und R⁷⁰ oder R⁷² und R⁷³ zusammen mit dem Stickstoffatom verbunden sein können, um einen
Ring zu bilden, und
X eine Gruppe bedeutet, die abgespalten werden kann, wenn die durch die Formel (XXXII) dargestellten Verbindungen mit einem nukleophilen Reagens reagieren.

22. Farbfotografisches Silberhalogenidmaterial nach Anspruch 1, worin der Härter gewählt ist aus Verbindungen, dargestellt durch die folgende Formel (XXXIII): worin R⁷⁴, R⁷⁵, R⁷⁶, R⁷⁷, R⁷⁸, und R⁷⁹, die gleich oder verschieden sein können, jeweils eine geradkettige oder verzweigte Alkylgruppe, eine Aralkylgruppe oder eine Arylgruppe bedeuten (R⁷⁴,
R⁷⁵, R⁷⁶, R⁷⁷, R⁷⁸ und R⁷⁹ können miteinander verbunden sein, um einen Ring zu bilden),
X eine Gruppe bedeutet, die abgespalten werden kann, wenn die durch die Formel (XXXIII) dargestellten Verbindungen mit einem nukleophilen Reagens reagieren, und
Y^{e} ein Anion bedeutet.

## Revendications

1. Matériau pour photographie en couleur à l'halogénure d'argent, qui comporte un durcisseur qui agit en activant un groupe carboxyle ainsi qu'au moins un coupleur polymère comprenant au moins un groupement répétitif de la formule suivante (I): où A représente un groupement polymère vinylique présentant un résidu formant coupleur chromogène capable de se coupler avec le produit résultant de l'oxydation d'un agent révélateur à base d'amine aromatique primaire, matériau caractérisé par le fait que ledit coupleur polymère comprend en outre au moins un groupement répétitif de la formule suivante (II): où B représente un groupement monomère vinylique présentant au moins un groupe choisi parmi un groupe amino et -COOM, dans lequel M représente un atome d'hydrogène, un métal alcalin ou l'ammonium, et par le fait que ledit coupleur polymère est soluble dans l'eau. Matériau pour photographie en couleur à l'halogénure d'argent de la revendication 1, dans lequel le groupement monomère représenté par la formule (1), capable de se coupler avec le produit résultant de l'oxydation d'un agent révélateur à base d'amine aromatique primaire pour former un colorant est représenté par la formule (III):
où R représente un atome d'hydrogène, un atome de chlore, ou un groupe alcoyle contenant de 1 à 4 atomes de carbone; D représente -COO-, -CONR'-, ou un groupe phényle ayant ou non fait l'objet d'une substitution; E représente un groupe alcoylène, un groupe phénylène ou un groupe aralcoylène, ayant ou non fait l'objet d'une substitution; F représente -CONR'-, -NR'CONR'-, -NR'COO-, -NR'CO-, -OCONR'-, -NR'-, -COO-, -OCO-, -CO-, -O-, -S0₂-, -NR'S0₂-, ou -S0₂NR'- dans lequel R' représente un atome d'hydrogène ou un groupe alcoyle ou un groupe aryle, ayant fait l'objet ou non l'objet d'une substitution, et, si deux ou plus R' se trouvent dans la même molécule, il peuvent être les mêmes ou différents;
1, m, et n sont 0 ou 1, sous réserve que 1, m et n ne soient pas 0 en même temps, et Q représente un résidu formant coupleur chromogène capable de se coupler avec le produit résultant de l'oxydation d'un agent révélateur à base d'amine aromatique primaire pour former un colorant. Matériau pour photographie en couleur à l'halogénure d'argent de la revendication 2, dans lequel le résidu formant coupleur chromogène représenté par Q, est choisi sous forme d'un résidu représenté par le type phénol (IV) ou (V) ou le type naphtol (VI) ou (VII) (un atome d'hydrogène autre que celui placé à la position de couplage ou celui du groupe OH placé en position numéro 1 se séparera pour se joindre avec F de la formule (III))
où R¹¹ représente un groupe capable de procéder à une substitution sur un composé cyclique phénolique ou un composé cyclique naphtolique ;
R¹² représente -CONR¹³R¹⁴, -NHCOR¹³, -NHCOOR¹⁵, -NHSO₂R¹⁵, -NYCONR¹³R¹⁴, ou -NHSO₂R¹³R¹⁴, dans lesquels R¹³ ou R¹⁴ représentent un atome d'hydrogène, un groupe aliphatique, un groupe aromatique, un groupe hétérocyclique, R15 représente un groupe aliphatique, un groupe aromatique, ou un groupe hétérocyclique, R¹³ et R¹⁴ peuvent être liés ensemble pour former un composé hétérocyclique;
p' est un entier de 0 à 3, q' est un entier de 0 à 2, r' et s' sont chacun des entiers de 0 à 4;
X représente un atome d'oxygène, un atome de soufre ou R¹⁶ N , dans lequel R¹⁶ représente un atome d'hydrogène ou un subtituant monovalent;
Z représente un atome d'hydrogène, ou un groupe qui peut se séparer lors de la réaction de couplage; et
Y représente un groupe d'atomes nécessaires pour former, avec l'atome de carbone, un composé cyclique à 5, 6 ou 7 membres.

4. Matériau pour photographie en couleur à l'halogènure d'argent de la revendication 2, dans lequel le résidu formant le coupleur chromogène représenté par Q est choisi sous forme d'un résidu représenté par les formules suivantes (VII), (VIII), (IX), (X), (XI), (XII) et (XIII), ces formules étant reliées à F de la formule (III) sur une portion quelconque de Ar, Z² et R²⁰ à _{R}³²
où Ar représente un substituant capable d'opérer une substitution à la première position d'un coupleur du type 2-pyrazoline-5-one;
R²⁰ représente un groupe anilino, ayant ou non subi une substitution, un groupe acylamino, ayant ou non subi une substitution, ou un groupe uréido, ayant ou non subi une substitution;
R²¹ R²², R²³, R²⁴, R²⁵, R²⁶, R²⁷, R²⁸, R²⁹, R³⁰, R³¹ et R³² représentent chacun un atome hydrogène, un groupe hydroxyle, un groupe alcoyle, ayant ou non subi une substitution, un groupe aryle, ayant ou non subi une substitution, un groupe hétérocyclique, ayant ou non subi une substitution, un groupe alcylamino, un groupe acylamino, un groupe anilino, un groupe alcoxycarbonyle, un groupe alcoylcar- bonyle, un groupe arylcarbonyle, un groupe alcoylthio, un groupe arylthio, un groupe carbamoyle, un groupe sulfamoyle ou un groupe sulfonamido; et
Z² représente un atome d'hydrogène ou un groupe qui peut se séparer lors de la réaction de couplage.

5. Matériau pour photographie en couleur à l'halogénure d'argent de la revendication 2, dans lequel le résidu formant coupleur chromogène représenté par Q est choisi sous forme d'un type pivaloylacétoa- nilido (XIV), ou d'un type benzoylacétoanilido (XV) ou (XVI)
où R³³, R³⁴, R³⁵ et R³⁶, qui peuvent être les mêmes ou différents, représentent chacun un atome d'hydrogène ou un substituant capable d'opérer une substitution dans le résidu d'un coupleur chromogène donnant le jaune et
Z³ représente un atome d'hydrogène ou un groupe qui peut se séparer lors d'une réaction de couplage.

. Matériau pour photographie en couleur à l'halogénure d'argent comme revendiqué dans la revendication 1, dans lequel le groupement monomère représenté par la formule (II) est choisi sous forme d'un groupement représenté par les formules suivantes (XXIVa) ou (XXIVb):
où R⁴⁵ représente un atome d'hydrogène, un groupe alcoyle d'ordre inférieur contenant de 1 à 4 atomes de carbone ou un atome de chlore; P représente -COO-, -CONHR⁴⁶'-, ou un groupe phénylène, ayant subi ou non une substitution; T représente -COO-, -CONH-, ou un groupe phénylène ayant subi ou non une substitution; L représente un groupe alcoylène, phénylène ou aralcoylène, ayant ou non subi une substitution; M représente un atome d'hydrogène, un métal alcalin ou l'ammonium; m' et n' représentent chacun 0 ou 1; et R⁴⁶ et R⁴⁶' représentent chacun un atome d'hydrogène ou un groupe alcoyle ou aryle ayant subi ou non une substitution.

7. Matériau pour photographie en couleur à l'halogénure d'argent de la revendication 1, dans lequel le coupleur polymère soluble dans l'eau contient un groupement monomère insaturé à liaison éthylénique, non chromogène, qui ne subit pas une réaction de couplage avec le produit résultant de l'oxydation d'un agent révélateur à base d'amine aromatique primaire, qui est autre que ceux représentés par les formules (I) et (II), et qui ne contient pas, dans la molécule, -COOM ou un groupe amino dans la proportion de 60% ou moins en termes du total des groupements monomères représentés par les formules (I) et (II).

8. Matériau pour photographie en couleur à l'halogènure d'argent de la revendication 7, dans lequel le groupement monomère insaturé à liaison éthylénique, non chromogène, autre que ceux représentés par les formules (I) et (II) est choisi parmi les esters d'acrylate, les esters de méthacrylate, les esters de crotonate, les esters vinyliques, les diesters de maléate, les diesters de fumarate, les diesters d'itaconate, les acrylamides, les méthacrylamides, les esters vinyliques et les styrènes.

9. Matériau pour photographie en couleur à l'halogènure d'argent de la revendication 1, dans lequel la proportion du groupement chromogène correspondant à la formule (L) dans le coupleur polymère est 5 à 80% en poids.

10. Matériau pour photographie en couleur à l'halogénure d'argent de la revendication 1, dans lequel la proportion du composant (groupement monomère) correspondant à la formule (II) dans le coupleur polymère est 20 à 95% en poids.

11. Matériau pour photographie en couleur à l'halogénure d'argent de la revendication 1, dans lequel on ajoute le coupleur polymère dans une proportion de 0,005 à 0,5 mole par mole d'argent, en termes du groupement monomère du coupleur représenté par la formule (1).

12. Matériau pour photographie en couleur à l'halogénure d'argent de la revendication 1, dans lequel le poids moléculaire du coupleur polymère est 5 x 10³ à 1 x 10⁷.

13. Matériau pour photographie en couleur à l'halogénure d'argent de la revendication 1, dans lequel le poids moléculaire équivalent du coupleur polymère est d'environ 250 à 4000.

14. Matériau pour photographie en couleur à l'halogénure d'argent de la revendication 1, dans lequel l'agent de durcissement est choisi parmi les composés représentés par la formule suivante (XXV):
où R⁴⁷ et R⁴⁸, qui peuvent être les mêmes ou différents, représentent chacun un groupe alcoyle, un groupe aryle, ou un groupe aralcoyle, dans lequel R⁴⁷ et R⁴⁸ peuvent être liés ensemble avec l'atome d'azote pour former un composé hétérocyclique, R⁴⁹ représente un substituant tel qu'un atome d'hydrogène, un atome d'halogène, un groupe carbamoyle, un groupe sulfo, un groupe uréido, un groupe alcoxy et un groupe alcoyle, et X^{e} représente un anion et devient un ion de comptage à l'égard du sel de N-carbamoylpyridinium.

15. Matériau pour photographie en couleur à l'halogénure d'argent de la revendication 1, dans lequel l'agent de durcissement est choisi parmi les composés représentés par la formule suivante (XXVI):
où R⁴⁷ et R⁴⁸, qui peuvent être les mêmes ou différents, représentent chacun un groupe alcoyle, un groupe aryle, ou un groupe aralcoyle, dans lequel R⁴⁷ et R⁴⁸ peuvent être liés ensemble avec l'atome d'azote pour former un composé hétérocyclique, R⁴⁹ représente un substituant tel qu'un atome d'hydrogène, un atome d'halogène, un groupe carbamoyle, un groupe sulfo, un groupe uréido, un groupe alcoxy et un groupe alcoyle, et X^{e} représente un anion et devient un ion de comptage à l'égard du sel de N-carbamoylpyridinium.

16. Matériau pour photographie en couleur à l'halogénure d'argent de la revendication 1, dans lequel l'agent de durcissement est choisi parmi les composés représentés par la formule suivante (XXVII):
où R⁵⁰, R⁵¹', R⁵² et R⁵³, qui peuvent être les mêmes ou différents, représentent chacun un groupe alcoyle, un groupe aralcoyle ou une groupe aryle dans lequel R⁵⁰, R⁵¹', 5⁵² et R⁵³ peuvent être liés ensemble pour former un composé cyclique,
X représente un groupe qui peut se séparer lorsque le composé représenté par le formule (XXVII) réagit avec un réactif nucléophile, et
Y^{e} représente un anion et, si Y^{e} représente un ion sulfonate, il peut se lier avec X, R⁵⁰, R⁵¹, R⁵² ou R⁵³ pour former un sel interne.

17. Matériau pour photographie en couleur à l'halogénure d'argent de la revendication 1, dans lequel l'agent de durcissement est choisi parmi les composés représentés par la formule suivante (XXVIII):
où R⁵⁴ représente un groupe alcoyle, un groupe cycloalcoyle, un groupe alcoxyalcoyle ou un groupe aralcoyle;
R^{54'} représente un groupe tel que défini pour R⁵⁴, ou
où R⁵⁵ représente un groupe alcoylène; R⁵⁶ et R⁵⁷, qui peuvent être les mêmes ou différents, représentent chacun un groupe alcoyle (R⁵⁴ et R⁵⁷ peuvent être liés ensemble avec l'atome d'azote pour former un composé hétérocyclique); R⁵⁸ représente un groupe alcoyle; X^{e} représente un anion et, si R⁵⁸ fait l'objet d'une substitution par un groupe sulfo, un sel interne se forme.

18. Matériau pour photographie en couleur à l'halogénure d'argent de la revendication 1, dans lequel l'agent de durcissement est choisi parmi les composés représentés par la formule suivante (XXIX):
où R⁵⁹ représente un groupe alcoyle, un groupe aryle ou un groupe aralcoyle, R⁶° et R⁶¹ qui peuvent être les mêmes ou différents, représentent chacun un substituant (R⁶° et R⁶¹ peuvent être liés ensemble avec le squelette du composé cyclique pyridinium pour former un composé cyclique condensé),
X représente un groupe qui peut se séparer lorsque les composés représentés par la formule (XXIX) réagissent avec un réactif nucléophile, et
Y^{e} représente un anion et si R⁵⁹ fait l'objet d'une substitution par un groupe sulfo, un sel interne se forme.

19. Matériau pour photographie en couleur à l'halogénure d'argent de la revendication 1 dans lequel l'agent de durcissement est choisi parmi les composés représentés par la formule suivante (XXX):
où R⁶³ et R⁶⁴, qui peuvent être les mêmes ou différents, représentent chacun un groupe alcoyle, un groupe aryle ou un groupe aralcoyle dans lequel R⁶³ et R⁶⁴ peuvent être reliés avec l'atome d'azote pour former un composé hétérocyclique, R⁶⁵ représente un groupe alcoyle, un groupe aryle ou un groupe aralcoyle et X^{e} représente un anion.

20. Matériau pour photographie en couleur à l'halogénure d'argent de la revendication 1, dans lequel l'agent de durcissement est choisi parmi les composés représentés par la formule suivante (XXXI):
où R⁶⁶ représente un groupe alcoyle à chaîne droite ou ramifiée, un groupe aralcoyle, un groupe aryle, un groupe alcényle ou un groupe hétéroaromatique et X représente un groupe qui peut se séparer lorsque les composés représentés par la formule (XXXI) réagissent avec un réactif nucléophile.

21. Matériau pour photographie en couleur à l'halogénure d'argent de la revendication 1, dans lequel l'agent de durcissement est choisi parmi les composés représentés par la formule suivante (XXXII):
où R⁶⁹ et R⁷⁰ représentent un groupe alcoyle à chaîne droite ou ramifiée, un groupe cycloalcoyle, un groupe aralcoyle, un groupe aryle, un groupe alcényle, ou un groupe hétérocyclique, R⁶⁹ et R⁷⁰ peunvent être reliés ensemble pour former un composé hétérocyclique;
R⁷¹ représente un groupe alcoyle à chaîne droite ou ramifiée, un groupe cycloalcoyle, un groupe aralcoyle, un groupe aryle, un groupe alcényle, un groupe hétérocyclique ou un groupe dans lequel R⁷² et R⁷³ représentent un groupe alcoyle à chaîne droite ou ramifiée, un groupe aralcoyle, un groupe aryle ou un groupe alcényle,
R⁶⁹ et R⁷⁰ ou R⁷² et R⁷³ peuvent être reliés ensemble avec l'atome d'azote pour former un composé cyclique, et
X représente un groupe qui peut se séparer lorsque les composés représentés par la formule (XXXII) réagissent avec un réactif nucléophile.

22. Matériau pour photographie en couleur à l'halogénure d'argent de la revendication 1, dans lequel l'agent de durcissement est choisi parmi les composés représentés par la formule suivante (XXXIII):
ou R⁷⁴, R⁷⁵, R⁷⁶, R⁷⁷, R⁷⁸ et R⁷⁹, qui peuvent être les mêmes ou différents, représentent chacun un groupe alcoyle à chaîne droite ou ramifiée, un groupe ^{aralcoyle,} un groupe aryle (^{R74, R75,} _{R76}, R⁷⁷, R⁷⁸ et R⁷⁹ peuvent être reliés ensemble pour former un composé cyclique),
X représente un groupe qui peut se séparer lorsque les composés représentés par la formule (XXXIII) réagissent avec un réactif nucléophile, et Y^{e} représente un anion.
